



US005516342A

# United States Patent [19]

Cherpeck

[11] Patent Number: 5,516,342

[45] Date of Patent: May 14, 1996

[54] FUEL ADDITIVE COMPOSITIONS  
CONTAINING POLY(OXYALKYLENE)  
HYDROXYAROMATIC ETHERS AND  
ALIPHATIC AMINES

[75] Inventor: Richard E. Cherpeck, Cotati, Calif.

[73] Assignee: Chevron Chemical Company, San  
Ramon, Calif.

[21] Appl. No.: 997,987

[22] Filed: Dec. 28, 1992

[51] Int. Cl. 6 C10L 1/18; C10L 1/22

[52] U.S. Cl. 44/347; 44/400; 44/442;  
44/443

[58] Field of Search 44/412, 434, 347,  
44/433, 443, 447, 448, 449, 450, 400, 432,  
442; 568/607, 608, 609, 610, 611, 606

## [56] References Cited

### U.S. PATENT DOCUMENTS

|           |         |                          |       |          |
|-----------|---------|--------------------------|-------|----------|
| 2,213,477 | 9/1940  | Steindorff et al.        | ..... | 568/606  |
| 2,984,553 | 5/1961  | Andress                  | ..... | 44/412   |
| 3,123,561 | 3/1964  | Rue                      | ..... | 568/609  |
| 3,438,757 | 4/1969  | Honnen et al.            | ..... | 44/433   |
| 3,443,918 | 5/1969  | Kautsky et al.           | ..... | 44/347   |
| 3,849,085 | 11/1974 | Kreuz et al.             | ..... | 44/78    |
| 4,123,232 | 10/1978 | Frost, Jr.               | ..... | 44/434   |
| 4,134,846 | 1/1979  | Machleder et al.         | ..... | 252/51.5 |
| 4,191,537 | 3/1980  | Lewis et al.             | ..... | 44/334   |
| 4,231,759 | 11/1980 | Udelhofen et al.         | ..... | 44/75    |
| 4,247,301 | 1/1981  | Honnen                   | ..... | 44/334   |
| 4,832,702 | 5/1989  | Kummer et al.            | ..... | 44/412   |
| 4,877,416 | 10/1989 | Campbell                 | ..... | 44/412   |
| 4,915,875 | 4/1990  | Diephouse et al.         | ..... | 568/607  |
| 5,024,678 | 6/1991  | Mertens-Gottselig et al. | ..... | 44/347   |
| 5,114,435 | 5/1992  | Abramo et al.            | ..... | 44/347   |
| 5,129,335 | 3/1993  | Cherpeck                 | ..... | 44/442   |
| 5,296,003 | 3/1994  | Cherpeck                 | ..... | 44/389   |
| 5,366,517 | 11/1994 | Cherpeck                 | ..... | 44/400   |
| 5,366,519 | 11/1994 | Cherpeck                 | ..... | 44/389   |
| 5,393,309 | 2/1995  | Cherpeck                 | ..... | 44/347   |

## FOREIGN PATENT DOCUMENTS

9212221 7/1992 WIPO

Primary Examiner—Jerry D. Johnson  
Attorney, Agent, or Firm—C. J. Caroli

## [57] ABSTRACT

A fuel additive composition comprising:

(a) a poly(oxyalkylene) hydroxyaromatic ether having the formula:



or a fuel-soluble salt thereof, where R<sub>1</sub> and R<sub>2</sub> are each independently hydrogen, hydroxy, lower alkyl having 1 to 6 carbon atoms, or lower alkoxy having 1 to 6 carbon atoms; R<sub>3</sub> and R<sub>4</sub> are each independently hydrogen or lower alkyl having 1 to 6 carbon atoms; R<sub>5</sub> is hydrogen, alkyl having 1 to 30 carbon atoms, phenyl, aralkyl or alkaryl having 7 to 36 carbon atoms, or an acyl group of the formula:



where R<sub>6</sub> is alkyl having 1 to 30 carbon atoms, phenyl, or aralkyl or alkaryl having 7 to 36 carbon atoms; n is an integer from 5 to 100; and x is an integer from 0 to 10; and

(b) an aliphatic amine having at least one basic nitrogen atom and containing a hydrocarbyl group which has sufficient molecular weight and carbon chain length to render the aliphatic amine soluble in hydrocarbons boiling in the gasoline or diesel range.

51 Claims, No Drawings

FUEL ADDITIVE COMPOSITIONS  
CONTAINING POLY(OXYALKYLENE)  
HYDROXYAROMATIC ETHERS AND  
ALIPHATIC AMINES

BACKGROUND OF THE INVENTION

1. Field of the Invention

This invention relates to a fuel additive composition. More particularly, this invention relates to a fuel additive composition containing a poly(oxyalkylene) hydroxyaromatic ether and an aliphatic amine.

2. Description of the Related Art

It is well known that automobile engines tend to form deposits on the surface of engine components, such as carburetor ports, throttle bodies, fuel injectors, intake ports and intake valves, due to the oxidation and polymerization of hydrocarbon fuel. These deposits, even when present in relatively minor amounts, often cause noticeable driveability problems, such as stalling and poor acceleration. Moreover, engine deposits can significantly increase an automobile's fuel consumption and production of exhaust pollutants. Therefore, the development of effective fuel detergents or "deposit control" additives to prevent or control such deposits is of considerable importance and numerous such materials are known in the art.

For example, aliphatic hydrocarbon-substituted phenols are known to reduce engine deposits when used in fuel compositions. U.S. Pat. No. 3,849,085, issued Nov. 19, 1974 to Kreuz et al., discloses a motor fuel composition comprising a mixture of hydrocarbons in the gasoline boiling range containing about 0.01 to 0.25 volume percent of a high molecular weight aliphatic hydrocarbon-substituted phenol in which the aliphatic hydrocarbon radical has an average molecular weight in the range of about 500 to 3,500. This patent teaches that gasoline compositions containing minor amount of an aliphatic hydrocarbon-substituted phenol not only prevent or inhibit the formation of intake valve and port deposits in a gasoline engine, but also enhance the performance of the fuel composition in engines designed to operate at higher operating temperatures with a minimum of decomposition and deposit formation in the manifold of the engine.

Similarly, U.S. Pat. No. 4,134,846, issued Jan. 16, 1979 to Machleider et al., discloses a fuel additive composition comprising a mixture of (1) the reaction product of an aliphatic hydrocarbon-substituted phenol, epichlorohydrin and a primary or secondary mono- or polyamine, and (2) a polyalkylene phenol. This patent teaches that such compositions show excellent carburetor, induction system and combustion chamber detergency and, in addition, provide effective rust inhibition when used in hydrocarbon fuels at low concentrations.

U.S. Pat. No. 4,231,759 discloses a fuel additive composition comprising the Mannich condensation product of (1) a high molecular weight sulfur-free alkyl-substituted hydroxyaromatic compound wherein the alkyl group has a number average molecular weight of about 600 to 3,000, (2) an amine containing at least one active hydrogen atom, and (3) an aldehyde, wherein the respective molar ratio of reactants is 1:0.1-10:0.1-10.

SUMMARY OF THE INVENTION

The present invention provides a novel fuel additive composition comprising:

(a) a poly(oxyalkylene) hydroxyaromatic ether having the formula:



or a fuel-soluble salt thereof; wherein R<sub>1</sub> and R<sub>2</sub> are each independently hydrogen, hydroxy, lower alkyl having 1 to 6 carbon atoms, or lower alkoxy having 1 to 6 carbon atoms; R<sub>3</sub> and R<sub>4</sub> are each independently hydrogen or lower alkyl having 1 to 6 carbon atoms; R<sub>5</sub> is hydrogen, alkyl having 1 to 30 carbon atoms, phenyl, aralkyl or alkaryl having 7 to 36 carbon atoms, or an acyl group of the formula:



wherein R<sub>6</sub> is alkyl having 1 to 30 carbon atoms, phenyl, or aralkyl or alkaryl having 7 to 36 carbon atoms; n is an integer from 5 to 100; and x is an integer from 0 to 10; and

25 (b) an aliphatic amine having at least one basic nitrogen atom and containing a hydrocarbyl group which has sufficient molecular weight and carbon chain length to render the aliphatic amine soluble in hydrocarbons boiling in the gasoline or diesel fuel range.

30 The present invention further provides a fuel composition comprising a major amount of hydrocarbons boiling in the gasoline or diesel range and an effective deposit-controlling amount of the novel fuel additive composition of the present invention.

35 The present invention additionally provides a fuel concentrate comprising an inert stable oleophilic organic solvent boiling in the range of from about 150° F. to 400° F. and from about 10 to 70 weight percent of the fuel additive composition of the present invention.

40 Among other factors, the present invention is based on the surprising discovery that the unique combination of a poly(oxyalkylene) hydroxyaromatic ether and an aliphatic amine provides excellent deposit control performance in internal combustion engines.

50 DETAILED DESCRIPTION OF THE  
INVENTION

55 As used herein the following terms have the following meanings unless expressly stated to the contrary.

The term "alkyl" refers to both straight- and branched-chain alkyl groups.

60 The term "lower alkyl" refers to alkyl groups having 1 to about 6 carbon atoms and includes primary, secondary and tertiary alkyl groups. Typical lower alkyl groups include, for example, methyl, ethyl, n-propyl, isopropyl, n-butyl, sec-butyl, t-butyl, n-pentyl, n-hexyl and the like.

65 The term "lower alkoxy" refers to the group —OR<sub>a</sub> wherein R<sub>a</sub> is lower alkyl. Typical lower alkoxy groups include methoxy, ethoxy, and the like.

The term "alkaryl" refers to the group:



wherein  $R_b$  and  $R_c$  are each independently hydrogen or an alkyl group, with the proviso that both  $R_b$  and  $R_c$  are not hydrogen. Typical alkaryl groups include, for example, tolyl, xylyl, cumenyl, ethylphenyl, butylphenyl, dibutylphenyl, hexylphenyl, octylphenyl, dioctylphenyl, nonylphenyl, decylphenyl, didecylphenyl, dodecylphenyl, hexadecylphenyl, octadecylphenyl, icosylphenyl, tricosylphenyl and the like. The term "alkylphenyl" refers to an alkaryl group of the above formula in which  $R_b$  is alkyl and  $R_c$  is hydrogen.

The term "aralkyl" refers to the group:



wherein  $R_d$  and  $R_e$  are each independently hydrogen or an alkyl group; and  $R_f$  is an alkylene group. Typical alkaryl groups include, for example, benzyl, methylbenzyl, dimethylbenzyl, phenethyl, and the like.

The term "hydrocarbyl" refers to an organic radical composed primarily of carbon and hydrogen which may be aliphatic, alicyclic, aromatic or combinations thereof, e.g., aralkyl or alkaryl. Such hydrocarbyl groups are generally relatively free of aliphatic unsaturation, i.e., olefinic or acetylenic unsaturation.

The term "oxyalkylene unit" refers to an ether moiety having the general formula:



wherein  $R_g$  and  $R_h$  are each independently hydrogen or lower alkyl groups.

The term "poly(oxyalkylene)" refers to a polymer or oligomer having the general formula:



wherein  $R_g$  and  $R_h$  are as defined above, and  $z$  is an integer greater than 1. When referring herein to the number of poly(oxyalkylene) units in a particular poly(oxyalkylene) compound, it is to be understood that this number refers to the average number of poly(oxyalkylene) units in such compounds unless expressly stated to the contrary.

#### The Poly(oxyalkylene) Hydroxyaromatic Ether

The poly(oxyalkylene) hydroxyaromatic ether component of the present invention has the general formula:



or a fuel-soluble salt thereof; wherein  $R_1$ ,  $R_2$ ,  $R_3$ ,  $R_4$ ,  $R_5$ ,  $n$  and  $x$  are as defined hereinabove.

Preferably,  $R_1$  is hydrogen, hydroxy, or lower alkyl having 1 to 4 carbon atoms. More preferably,  $R_1$  is hydrogen or hydroxy. Most preferably,  $R_1$  is hydrogen.

$R_2$  is preferably hydrogen.

Preferably, one of  $R_3$  and  $R_4$  is lower alkyl having 1 to 3 carbon atoms and the other is hydrogen. More preferably, one of  $R_3$  and  $R_4$  is methyl or ethyl and the other is hydrogen. Most preferably, one of  $R_3$  and  $R_4$  is ethyl and the other is hydrogen.

10  $R_5$  is preferably hydrogen, alkyl having 2 to 22 carbon atoms, alkylphenyl having an alkyl group containing 4 to 24 carbon atoms, or an acyl group having the formula:  $-\text{C}(\text{O})\text{R}_7$ , wherein  $R_7$  is alkyl having 4 to 12 carbon atoms. More preferably,  $R_5$  is hydrogen, alkyl having 4 to 12 carbon atoms, or alkylphenyl having an alkyl group containing 4 to 12 carbon atoms. Most preferably,  $R_5$  is hydrogen.

15 Preferably,  $n$  is an integer from 10 to 50. More preferably,  $n$  is an integer from 15 to 30. Preferably,  $x$  is an integer from 0 to 2. More preferably,  $x$  is 0.

20 A preferred group of poly(oxyalkylene) hydroxyaromatic ethers for use in this invention are those of formula I wherein  $R_1$  is hydrogen, hydroxy, or lower alkyl having 1 to 4 carbon atoms;  $R_2$  is hydrogen; one of  $R_3$  and  $R_4$  is hydrogen and the other is methyl or ethyl;  $R_5$  is hydrogen, alkyl having 4 to 12 carbon atoms, alkylphenyl having an alkyl group containing 4 to 12 carbon atoms, or an acyl group having the formula:  $-\text{C}(\text{O})\text{R}_7$ , wherein  $R_7$  is alkyl having 4 to 12 carbon atoms;  $n$  is 15 to 30 and  $x$  is 0.

25 Another preferred group of poly(oxyalkylene) hydroxyaromatic ethers for use in this invention are those of formula I wherein  $R_1$  is hydrogen, hydroxy, or lower alkyl having 1 to 4 carbon atoms;  $R_2$  is hydrogen; one of  $R_3$  and  $R_4$  is hydrogen and the other is methyl or ethyl;  $R_5$  is hydrogen, alkyl having 4 to 12 carbon atoms, alkylphenyl having an alkyl group containing 4 to 12 carbon atoms, or an acyl group having the formula:  $-\text{C}(\text{O})\text{R}_7$ , wherein  $R_7$  is alkyl having 4 to 12 carbon atoms;  $n$  is 15 to 30 and  $x$  is 1 or 2.

30 35 A more preferred group of poly(oxyalkylene) hydroxyaromatic ethers for use in this invention are those of formula I wherein  $R_1$  is hydrogen or hydroxy;  $R_2$  is hydrogen; one of  $R_3$  and  $R_4$  is hydrogen and the other is methyl or ethyl;  $R_5$  is hydrogen, alkyl having 4 to 12 carbon atoms, or alkylphenyl having an alkyl group containing 4 to 12 carbon atoms;  $n$  is 15 to 30; and  $x$  is 0.

40 45 A particularly preferred group of poly(oxyalkylene) hydroxyaromatic ethers for use in this invention are those having the formula:



50 whereon one of  $R_8$  and  $R_9$  is methyl or ethyl and the other is hydrogen; and  $m$  is an integer from 15 to 30.

55 60 The poly(oxyalkylene) hydroxyaromatic ether component of the present fuel additive composition will generally have a sufficient molecular weight so as to be non-volatile at normal engine intake valve operating temperatures (about 200°-250° C.). Typically, the molecular weight of the poly(oxyalkylene) hydroxyaromatic ether component will range from about 600 to about 10,000, preferably from 1,000 to 3,000.

65 65 Generally, the poly(oxyalkylene) hydroxyaromatic ethers employed in this invention will contain an average of about 5 to about 100 oxyalkylene units; preferably, 10 to 50 oxyalkylene units; more preferably, 15 to 30 oxyalkylene units.

Fuel-soluble salts of poly(oxyalkylene) hydroxyaromatic ethers are also contemplated to be useful in the fuel additive composition of the present invention. Such salts include alkali metal, alkaline earth metal, ammonium, substituted ammonium and sulfonium salts. Preferred metal salts are the alkali metal salts, particularly the sodium and potassium salts, and the substituted ammonium salts, particularly tetraalkyl-substituted ammonium salts, such as the tetrabutylammonium salts.

### General Synthetic Procedures

The poly(oxyalkylene) hydroxyaromatic ether component of the present fuel additive composition may be prepared by the following general methods and procedures. It should be appreciated that where typical or preferred process conditions (e.g. reaction temperatures, times, mole ratios of reactants, solvents, pressures, etc.) are given, other process conditions may also be used unless otherwise stated. Optimum reaction conditions may vary with the particular reactants or solvents used, but such conditions can be determined by one skilled in the art by routine optimization procedures.

The poly(oxyalkylene) hydroxyaromatic ethers employed in the present fuel additive composition may be prepared from a hydroxyaromatic compound having the formula:



wherein R<sub>1</sub>, R<sub>2</sub>, and x are as defined above.

The hydroxyaromatic compounds of formula III are either known compounds or can be prepared from known compounds by conventional procedures. Suitable hydroxyaromatic compounds for use as starting materials in this invention include catechol, resorcinol, hydroquinone, 1,2,3-trihydroxybenzene (pyrogallol), 1,2,4-trihydroxybenzene (hydroquinol), 1,3,5-trihydroxybenzene (phloroglucinol), 1,4-dihydroxy-2-methylbenzene, 1,3-dihydroxy-5-methylbenzene, 2-t-butyl-1,4-dihydroxybenzene, 2,6-di-t-butyl-1,4-dihydroxybenzene, 1,4-dihydroxy-2-methoxybenzene, 1,3-dihydroxy-5-methoxybenzene, 4-hydroxybenzyl alcohol, 4-hydroxyphenethyl alcohol and the like.

In a preferred method of synthesizing the poly(oxyalkylene) hydroxyaromatic ether component of the present fuel additive composition, a hydroxyaromatic compound of formula III is first selectively protected to provide a compound having the formula:



wherein R<sub>10</sub> is a suitable hydroxyl protecting group, such as benzyl, tert-butyldimethylsilyl, methoxymethyl, and the like; R<sub>11</sub> and R<sub>12</sub> are each independently hydrogen, lower alkyl, lower alkoxy, or the group —OR<sub>13</sub>, wherein R<sub>13</sub> is a suitable hydroxyl protecting group, such as benzyl, tert-butyldimethylsilyl, methoxymethyl, and the like. Preferably, R<sub>10</sub> and R<sub>13</sub> are benzyl; except in the case where x is 1, then R<sub>10</sub> and R<sub>13</sub> are preferably a tert-butyldimethylsilyl group.

Selective protection of III may be accomplished using conventional procedures. The choice of a suitable protecting group for a particular hydroxyaromatic compound will be apparent to those skilled in the art. Various protecting groups, and their introduction and removal, are described, for example, in T. W. Greene and P. G. M. Wuts, *Protective Groups in Organic Synthesis*, Second Edition, Wiley, New York, 1991, and references cited therein. Alternatively, the protected derivatives IV can be prepared from known starting materials other than the hydroxyaromatic compounds of formula III by conventional procedures. In some cases, the protected derivatives IV are commercially available, e.g. 4-benzyloxyphenol is commercially available from Aldrich Chemical Co., Milwaukee, Wis. 53233.

The protected hydroxyaromatic compound of formula IV is then deprotonated with a suitable base to provide a metal salt having the formula:



wherein R<sub>10</sub>, R<sub>11</sub>, R<sub>12</sub> and x are as defined above; and M is a metal cation, such as lithium, sodium or potassium.

Generally, this deprotonation reaction will be effected by contacting IV with a strong base, such as sodium hydride, potassium hydride, sodium amide and the like, in an inert solvent, such as toluene, xylene and the like, under substantially anhydrous conditions at a temperature in the range from about -10° C. to about 120° C. for about 0.25 to about 3 hours.

Metal salt V is generally not isolated, but is reacted in situ with about 5 to about 100 molar equivalents of an alkylene oxide (an epoxide) having the formula:



wherein R<sub>3</sub> and R<sub>4</sub> are as defined above, to provide, after neutralization, a poly(oxyalkylene) polymer or oligomer having the formula:



wherein R<sub>3</sub>, R<sub>4</sub>, R<sub>10</sub>, R<sub>11</sub>, R<sub>12</sub>, n and x are as defined above.

Typically, this polymerization reaction is conducted in a substantially anhydrous inert solvent at a temperature of about 30° C. to about 150° C. for about 2 to about 120 hours.

Suitable solvents for this reaction, include toluene, xylene and the like. The reaction will generally be conducted at a pressure sufficient to contain the reactants and the solvent, preferably at atmospheric or ambient pressure. More detailed reaction conditions for preparing poly(oxyalkylene) compounds may be found in U.S. Pat. Nos. 2,782,240 and 2,841,479, which are incorporated herein by reference.

The amount of alkylene oxide employed in this reaction will depend on the number of oxyalkylene units desired in the product. Typically, the molar ratio of alkylene oxide VI to metal salt V will range from about 5:1 to about 100:1; preferably, from 10:1 to 50:1, more preferably from 15:1 to 30:1.

Suitable alkylene oxides for use in the polymerization reaction include, for example, ethylene oxide; propylene oxide; butylene oxides, such as 1,2-butylene oxide (1,2-epoxybutane) and 2,3-butylene oxide (2,3-epoxybutane); pentylene oxides; hexylene oxides; octylene oxides and the like. Preferred alkylene oxides are propylene oxide and 1,2-butylene oxide.

In the polymerization reaction, a single type of alkylene oxide may be employed, e.g. propylene oxide, in which case the product is a homopolymer, e.g. a poly(oxypropylene). However, copolymers are equally satisfactory and random copolymers are readily prepared by contacting the metal salt V with a mixture of alkylene oxides, such as a mixture of propylene oxide and 1,2-butylene oxide, under polymerization conditions. Copolymers containing blocks of oxyalkylene units are also suitable for use in the present invention. Block copolymers may be prepared by contacting the metal salt V with first one alkylene oxide, then others in any order, or repetitively, under polymerization conditions.

Poly(oxyalkylene) polymers of formula VII may also be prepared by living or immortal polymerization as described by S. Inoue and T. Aida in *Encyclopedia of Polymer Science and Engineering*, Second Edition, Supplemental Volume, J. Wiley and Sons, New York, pages 412-420 (1989). These procedures are especially useful for preparing poly(oxyalkylene) alcohols of formula V in which R<sub>3</sub> and R<sub>4</sub> are both alkyl groups.

Deprotection of the aromatic hydroxyl group(s) of VII using conventional procedures provides a poly(oxyalkylene) hydroxyaromatic ether having the formula:



wherein R<sub>1</sub>-R<sub>4</sub>, n and x are as defined above.

Appropriate conditions for this deprotection step will depend upon the protecting group(s) utilized in the synthesis and will be readily apparent to those skilled in the art. For example, benzyl protecting groups may be removed by hydrogenolysis under 1 to about 4 atmospheres of hydrogen in the presence of a catalyst, such as palladium on carbon. Typically, this deprotection reaction will be conducted in an inert solvent, preferably a mixture of ethyl acetate and acetic acid, at a temperature of from about 0° C. to about 40° C. for about 1 to about 24 hours.

The poly(oxyalkylene) hydroxyaromatic ethers employed in the present fuel additive composition that contain an alkyl or aralkyl ether moiety, i.e. those having the formula:



wherein R<sub>1</sub>-R<sub>4</sub>, n and x are as defined above, and R<sub>14</sub> is an alkyl group or aralkyl group, may be conveniently prepared from a compound of formula VIII by selectively alkylating the hydroxyl group of the poly(oxyalkylene) moiety of VIII with a suitable alkylating agent.

Typically, this alkylation reaction will be conducted by first contacting VIII with a sufficient amount of a strong base capable of abstracting a proton from each the hydroxyl

groups present in VIII, including the aromatic hydroxyl group(s) and the hydroxyl group of the poly(oxyalkylene) moiety. Suitable bases for this reaction include, for example, sodium hydride, potassium hydride, sodium amide and the like. Generally, this deprotonation reaction will be conducted in an inert solvent, such as toluene, tetrahydrofuran, and the like, under substantially anhydrous conditions at a temperature in the range from -10° C. to 120° C. for about 0.25 to about 3 hours. The resulting metal salt is then contacted with about 0.90 to about 1.1 molar equivalents of a suitable alkylating agent at a temperature in the range from 0° C. to 120° C. for about 1 to about 50 hours to afford, after neutralization, a poly(oxyalkylene) hydroxyaromatic ether of formula IX.

Suitable alkylating agents for use in this reaction include alkyl and aralkyl halides, such as alkyl chlorides, bromides and iodides and aralkyl chlorides, bromides and iodides; and alkyl and aralkyl sulfonates, such as alkyl mesylates and tosylates, and aralkyl mesylates and tosylates.

Preferred alkylating agents are primary and secondary alkyl halides having 1 to 30 carbon atoms, and primary and secondary aralkyl halides having 7 to 36 carbon atoms; more preferred alkylating agents are primary alkyl halides having 4 to 12 carbon atoms.

Representative examples of alkylating agents include, but are not limited to, methyl iodide, ethyl iodide, n-propyl bromide, n-butyl bromide, n-pentyl bromide, n-hexyl chloride, n-octyl chloride, n-decyl chloride, benzyl chloride and phenethyl chloride. Particularly preferred alkylating agents are benzyl chloride, n-butyl bromide.

Alternatively, poly(oxyalkylene) hydroxyaromatic ethers of formula IX may be prepared by alkylating the hydroxyl group of the poly(oxyalkylene) moiety of protected intermediate VII, and then deprotecting the resulting product. The conditions for alkylating intermediate VII are essentially the same as those described above; however, a lesser amount of base will be required since the aromatic hydroxyl groups of VII are in a protected form.

Other suitable methods for preparing alkyl and alkaryl ethers from alcohols, and appropriate reaction conditions for such reactions, can be found, for example, in I. T. Harrison and S. Harrison, *Compendium of Organic Synthetic Methods*, Vol. 1, pp. 310-312, Wiley-Interscience, New York (1971) and references cited therein.

The poly(oxyalkylene) hydroxyaromatic ethers employed in the present fuel additive composition that contain an alkaryl ether moiety, i.e. those having the formula:



wherein R<sub>1</sub>-R<sub>4</sub>, n and x are as defined above, and R<sub>15</sub> is a phenyl or alkaryl group, may be prepared from intermediate VII in several steps by first converting the hydroxyl group present of the poly(oxyalkylene) moiety of VII into a suitable leaving group, i.e. forming an intermediate having the formula:



wherein  $R_3$ ,  $R_4$ ,  $R_{10}$ ,  $R_{11}$ ,  $R_{12}$ ,  $n$  and  $x$  are as defined above, and  $W$  is a suitable leaving group; and then displacing the leaving group of XI with a metal salt of a phenol having the formula:



wherein  $R_{16}$  and  $R_{17}$  are each independently hydrogen or an alkyl group. Subsequent deprotection of the resulting product affords poly(oxyalkylene) hydroxyaromatic ethers of formula X.

The hydroxyl group of the poly(oxyalkylene) moiety of VII may be converted into a suitable leaving group by contacting VII with a sulfonyl chloride to form a sulfonate ester, such as a methanesulfonate (mesylate) or a toluene-sulfonate (tosylate). Typically, this reaction is conducted in the presence of a suitable amine, such as triethylamine or pyridine, in an inert solvent, such as dichloromethane, at a temperature in the range of about  $-10^\circ C$ . to about  $30^\circ C$ . Alternatively, the hydroxyl group of the poly(oxyalkylene) moiety of VII can be exchanged for a halide, such chloride or bromide, by contacting VII with a halogenating agent, such as thionyl chloride, oxalyl chloride or phosphorus tribromide. Other suitable methods for preparing sulfonates and halides from alcohols, and appropriate reaction conditions for such reactions, can be found, for example, in I. T. Harrison and S. Harrison, *Compendium of Organic Synthetic Methods*, Vol. 1, pp. 331-337, Wiley-Interscience, New York (1971) and references cited therein.

After forming intermediate XI, the leaving group may be displaced therefrom by contacting XI with metal salt XII. Generally, this reaction will be conducted in an inert solvent, such as toluene, tetrahydrofuran and the like, under substantially anhydrous conditions at a temperature in the range of about  $25^\circ C$ . to about  $150^\circ C$ . for about 1 to about 48 hours. The metal salt XII can be formed by contacting the corresponding phenol with a strong base capable of abstracting the proton from the phenolic hydroxyl group, such as sodium hydride, potassium hydride, sodium amide and the like, in an inert solvent.

Suitable phenolic compounds for use in this reaction include phenol, monoalkyl-substituted phenols and dialkyl-substituted phenols. Monoalkyl-substituted phenols are preferred, especially monoalkylphenols having an alkyl substituent in the para position. Representative examples of suitable phenolic compounds include, but are not limited to, phenol, methylphenol, dimethylphenol, ethylphenol, butylphenol, octylphenol, decylphenol, dodecylphenol, tetradecylphenol, hexadecylphenol, octadecylphenol, eicosylphenol, tetracosylphenol, hexacosylphenol, triacontylphenol and the like. Also, mixtures of alkylphenols may be employed, such as a mixture of  $C_{14}$ - $C_{18}$  alkylphenols, a mixture of  $C_{18}$ - $C_{24}$  alkylphenols, a mixture of  $C_{20}$ - $C_{24}$  alkylphenols, or a mixture of  $C_{16}$ - $C_{26}$  alkylphenols.

Particularly preferred alkylphenols are those derived from alkylation of phenol with polymers or oligomers of  $C_3$  to  $C_6$  olefins, such as polypropylene or polybutene. These poly-

mers preferably contain 10 to 30 carbon atoms. An especially preferred alkylphenol is prepared by alkylating phenol with a propylene polymer having an average of 4 units. This polymer has the common name of propylene tetramer and is commercially available.

Alternatively, the poly(oxyalkylene) hydroxyaromatic ethers of formula X can be prepared by displacing a leaving group from an intermediate having the formula:



wherein  $R_3$ ,  $R_4$ ,  $R_{15}$ ,  $n$  and  $x$  are as defined above, and  $W$  is a suitable leaving group, with metal salt V; and then deprotecting the resulting product. Conditions for this reaction are essentially the same as those described above for reaction of XI with XII. Compounds of formula XIII may be prepared from XII and VI using the conditions described above for the preparation of VII, followed by conversion of the hydroxyl group of the poly(oxyalkylene) moiety of the resulting product into a suitable leaving using the procedures described above for the preparation of XI.

The poly(oxyalkylene) hydroxyaromatic ethers employed in the present fuel additive composition that contain an acyl moiety, i.e those having the formula:



wherein  $R_1$ - $R_4$ ,  $R_6$ ,  $n$  and  $x$  are as defined above; may be prepared from intermediate VII by first acylating the hydroxyl group of the poly(oxyalkylene) moiety of VII to form an ester. Subsequent deprotection of the aromatic hydroxyl group(s) of the resulting ester using conventional procedures then affords poly(oxyalkylene) hydroxyaromatic ethers of formula XIV.

Generally, the acylation reaction will be conducted by contacting intermediate VII with about 0.95 to about 1.2 molar equivalents of a suitable acylating agent. Suitable acylating agents for use in this reaction include acyl halides, such as acyl chlorides and bromides; and carboxylic acid anhydrides. Preferred acylating agents are those having the formula:  $R_6C(O)-X$ , wherein  $R_6$  is alkyl having 1 to 30 carbon atoms, phenyl, or aralkyl or alkaryl having 7 to 36 carbon atoms, and  $X$  is chloro or bromo. More preferred acylating agents are those having the formula:  $R_7C(O)-X$ , wherein  $R_7$  is alkyl having 4 to 12 carbon atoms. Representative examples of suitable acylating agents include, but are not limited to, acetyl chloride, acetic anhydride, propionyl chloride, butanoyl chloride, pivaloyl chloride, octanoyl chloride, decanoyl chloride 4-t-butylbenzoyl chloride and the like.

Generally, this reaction is conducted in an inert solvent, such as toluene, dichloromethane, diethyl ether and the like, at a temperature in the range of about  $25^\circ C$ . to about  $150^\circ C$ . and is generally complete in about 0.5 to about 48 hours. When an acyl halide is employed as the acylating agent, this reaction is preferably conducted in the presence of a sufficient amount of an amine capable of neutralizing the acid generated during the reaction, such as triethylamine, di(isopropyl)ethylamine, pyridine or 4-dimethylaminopyridine.

Additional methods for preparing esters from alcohols, and suitable reaction conditions for such reactions, can be found, for example, in I. T. Harrison and S. Harrison,

*Compendium of Organic Synthetic Methods*, Vol. 1, pp. 273-276 and 280-283, Wiley-Interscience, New York (1971) and references cited therein.

### The Aliphatic Amine

The aliphatic amine component of the present fuel additive composition is an aliphatic amine having at least one basic nitrogen atom and containing a hydrocarbyl group which has sufficient molecular weight and carbon chain length to render the aliphatic amine soluble in hydrocarbons boiling in the gasoline or diesel range. Preferably, such aliphatic amines will also be of sufficient molecular weight so as to be nonvolatile at normal engine intake valve operating temperatures, generally in the range of about 175° C. to 300° C.

In general, the aliphatic amine will contain a hydrocarbyl group having a number average molecular weight in the range of about 250 to 3,000, preferably in the range of about 700 to 2,200, and more preferably, in the range of about 900 to 1,500.

In a preferred embodiment, the aliphatic amine component of the present fuel additive composition is a fuel-soluble aliphatic amine selected from the group consisting of:

- (1) a straight or branched chain hydrocarbyl-substituted amine having at least one basic nitrogen atom wherein the hydrocarbyl group has a number average molecular weight of about 250 to 3,000,
- (2) a hydroxyalkyl-substituted amine comprising the reaction product of (i) a polyolefin epoxide derived from a branched-chain polyolefin having a number average molecular weight of about 250 to 3,000, and (ii) a nitrogen-containing compound selected from ammonia, a monoamine having from 1 to 40 carbon atoms, and a polyamine having from 2 to about 12 amine nitrogen atoms and from 2 to about 40 carbon atoms, and
- (3) a straight or branched chain hydrocarbyl-substituted succinimide comprising the reaction product of a straight or branched chain hydrocarbyl-substituted succinic acid or anhydride, wherein the hydrocarbyl group has a number average molecular weight of about 250 to 3,000, and a polyamine having from 2 to about 12 amine nitrogen atoms and 2 to about 40 carbon atoms.

#### A. The Hydrocarbyl-Substituted Amine

The hydrocarbyl-substituted amine employed as the aliphatic amine component of the present fuel additive composition is a straight or branched chain hydrocarbyl-substituted amine having at least one basic nitrogen atom wherein the hydrocarbyl group has a number average molecular weight of about 250 to 3,000.

Preferably, the hydrocarbyl group will have a number average molecular weight in the range of about 700 to 2,200, and more preferably, in the range of about 900 to 1,500. The hydrocarbyl group may be either straight chain or branched chain. When the hydrocarbyl group is straight chain, a preferred aliphatic amine is oleyl amine.

When employing a branched chain hydrocarbyl amine, the hydrocarbyl group is preferably derived from polymers of C<sub>2</sub> to C<sub>6</sub> olefins. Such branched-chain hydrocarbyl group will ordinarily be prepared by polymerizing olefins of from 2 to 6 carbon atoms (ethylene being copolymerized with another olefin so as to provide a branched-chain). The branched chain hydrocarbyl group will generally have at least 1 branch per 6 carbon atoms along the chain, preferably

at least 1 branch per 4 carbon atoms along the chain and, more preferably, at least 1 branch per 2 carbon atoms along the chain. The preferred branched-chain hydrocarbyl groups are polypropylene and polyisobutylene. The branches will usually be of from 1 to 2 carbon atoms, preferably 1 carbon atom, that is, methyl. In general, the branched-chain hydrocarbyl group will contain from about 18 to about 214 carbon atoms, preferably from about 50 to about 157 carbon atoms.

In most instances, the branched-chain hydrocarbyl amines are not a pure single product, but rather a mixture of compounds having an average molecular weight. Usually, the range of molecular weights will be relatively narrow and peaked near the indicated molecular weight.

The amine component of the branched-chain hydrocarbyl amines may be derived from ammonia, a monoamine or a polyamine. The monoamine or polyamine component embodies a broad class of amines having from 1 to about 12 amine nitrogen atoms and from 1 to 40 carbon atoms with a carbon to nitrogen ratio between about 1:1 and 10:1. Generally, the monoamine will contain from 1 to about 40 carbon atoms and the polyamine will contain from 2 to about 12 amine nitrogen atoms and from 2 to about 40 carbon atoms. In most instances, the amine component is not a pure single product, but rather a mixture of compounds having a major quantity of the designated amine. For the more complicated polyamines, the compositions will be a mixture of amines having as the major product the compound indicated and having minor amounts of analogous compounds. Suitable monoamines and polyamines are described more fully below in the discussion of hydroxyalkyl-substituted amines.

When the amine component is a polyamine, it will preferably be a polyalkylene polyamine, including alkylene diamine. Preferably, the alkylene group will contain from 2 to 6 carbon atoms, more preferably from 2 to 3 carbon atoms. Examples of such polyamines include ethylene diamine, diethylene triamine, triethylene tetramine and tetraethylene pentamine. Preferred polyamines are ethylene diamine and diethylene triamine.

A particularly preferred branched-chain hydrocarbyl amine is polyisobutyl ethylene diamine.

The branched-chain hydrocarbyl amines employed in the fuel additive composition of the invention are prepared by conventional procedures known in the art. Such branched-chain hydrocarbyl amines and their preparations are described in detail in U.S. Pat. Nos. 3,438,757; 3,565,804; 3,574,576; 3,848,056 and 3,960,515, the disclosures of which are incorporated herein by reference.

#### B. The Hydroxyalkyl-Substituted Amine

The hydroxyalkyl-substituted amine additive employed in the fuel composition of the present invention comprises the reaction product of (a) a polyolefin epoxide derived from a branched chain polyolefin having an average molecular weight of about 250 to 3,000 and (b) a nitrogen-containing compound selected from ammonia, a monoamine having from 1 to 40 carbon atoms, and a polyamine having from 2 to about 12 amine nitrogen atoms and from 2 to about 40 carbon atoms. The amine component of this reaction product is selected to provide solubility in the fuel composition and deposit control activity.

#### Polyolefin Epoxide Component

The polyolefin epoxide component of the presently employed hydroxyalkyl-substituted amine reaction product is obtained by oxidizing a polyolefin with an oxidizing agent to give an alkylene oxide, or epoxide, in which the oxirane

ring is derived from oxidation of the double bond in the polyolefin.

The polyolefin starting material used in the preparation of the polyolefin epoxide is a high molecular weight branched chain polyolefin having an average molecular weight of about 250 to 3,000, preferably from about 700 to 2,200, and more preferably from about 900 to 1,500.

Such high molecular weight polyolefins are generally mixtures of molecules having different molecular weights and can have at least one branch per 6 carbon atoms along the chain, preferably at least one branch per 4 carbon atoms along the chain, and particularly preferred that there be about one branch per 2 carbon atoms along the chain. These branched chain olefins may conveniently comprise polyolefins prepared by the polymerization of olefins of from 2 to 6 carbon atoms, and preferably from olefins of from 3 to 4 carbon atoms, and more preferably from propylene or isobutylene. When ethylene is employed, it will normally be copolymerized with another olefin so as to provide a branched chain polyolefin. The addition-polymerizable olefins employed are normally 1-olefins. The branch may be of from 1 to 4 carbon atoms, more usually of from 1 to 2 carbon atoms, and preferably methyl.

In general, any high molecular weight branched chain polyolefin isomer whose epoxide is capable of reacting with an amine is suitable for use in preparing the presently employed fuel additives. However, sterically hindered epoxides, such as tetra-alkyl substituted epoxides, are generally slower to react.

Particularly preferred polyolefins are those containing an alkylvinylidene isomer present in an amount at least about 20%, and preferably at least 50%, of the total polyolefin composition. The preferred alkylvinylidene isomers include methylvinylidene and ethylvinylidene, more preferably the methylvinylidene isomer.

The especially preferred high molecular weight polyolefins used to prepare the instant polyolefin epoxides are polyisobutenes which comprise at least about 20% of the more reactive methylvinylidene isomer, preferably at least 50% and more preferably at least 70%. Suitable polyisobutenes include those prepared using  $BF_3$  catalysts. The preparation of such polyisobutenes in which the methylvinylidene isomer comprises a high percentage of the total composition is described in U.S. Pat. Nos. 4,152,499 and 4,605,808.

Examples of suitable polyisobutenes having a high alkylvinylidene content include Ultravis 30, a polyisobutene having a molecular weight of about 1300 and a methylvinylidene content of about 76%, available from British Petroleum.

As noted above, the polyolefin is oxidized with a suitable oxidizing agent to provide an alkylene oxide, or polyolefin epoxide, in which the oxirane ring is formed from oxidation of the polyolefin double bond.

The oxidizing agent employed may be any of the well known conventional oxidizing agents used to oxidize double bonds. Suitable oxidizing agents include hydrogen peroxide, peracetic acid, perbenzoic acid, performic acid, monoperphthalic acid, percamphoric acid, persuccinic acid and perfluoroacetic acid. The preferred oxidizing agent is peracetic acid.

When peracetic acid is used as the oxidizing agent, generally a 40% peracetic acid solution and about a 5% equivalent of sodium acetate (as compared to the peracetic acid) is added to the polyolefin in a molar ratio of peracid to olefin in the range of about 1.5:1 to 1:1, preferably about

1.2:1. The mixture is gradually allowed to react at a temperature in the range of about 20° C. to 90° C.

The resulting polyolefin epoxide, which is isolated by conventional techniques, is generally a liquid or semi-solid resin at room temperature, depending on the type and molecular weight of olefin employed.

#### Amine Component

The amine component of the presently employed hydroxyalkyl-substituted amine reaction product is derived from a nitrogen-containing compound selected from ammonia, a monoamine having from 1 to 40 carbon atoms, and a polyamine having from 2 to about 12 amine nitrogen atoms and from 2 to about 40 carbon atoms. The amine component is reacted with a polyolefin epoxide to produce the hydroxyalkyl-substituted amine fuel additive finding use within the scope of the present invention. The amine component provides a reaction product with, on the average, at least about one basic nitrogen atom per product molecule, i.e., a nitrogen atom titratable by a strong acid.

Preferably, the amine component is derived from a polyamine having from 2 to about 12 amine nitrogen atoms and from 2 to about 40 carbon atoms. The polyamine preferably has a carbon-to-nitrogen ratio of from about 1:1 to 10:1.

The polyamine may be substituted with substituents selected from (A) hydrogen, (B) hydrocarbyl groups of from 1 to about 10 carbon atoms, (C) acyl groups of from 2 to about 10 carbon atoms, and (D) monoketo, monohydroxy, mononitro, monocyno, lower alkyl and lower alkoxy derivatives of (B) and (C). "Lower", as used in terms like lower alkyl or lower alkoxy, means a group containing from 1 to about 6 carbon atoms. At least one of the substituents on one of the basic nitrogen atoms of the polyamine is hydrogen, e.g., at least one of the basic nitrogen atoms of the polyamine is a primary or secondary amino nitrogen.

Hydrocarbyl, as used in describing the amine components of this invention, denotes an organic radical composed of carbon and hydrogen which may be aliphatic, alicyclic, aromatic or combinations thereof, e.g., aralkyl. Preferably, the hydrocarbyl group will be relatively free of aliphatic unsaturation, i.e., ethylenic and acetylenic, particularly acetylenic unsaturation. The substituted polyamines of the present invention are generally, but not necessarily, N-substituted polyamines. Exemplary hydrocarbyl groups and substituted hydrocarbyl groups include alkyls such as methyl, ethyl, propyl, butyl, isobutyl, pentyl, hexyl, octyl, etc., alkenyls such as propenyl, isobutenyl, hexenyl, octenyl, etc., hydroxyalkyls, such as 2-hydroxyethyl, 3-hydroxypropyl, hydroxy-isopropyl, 4-hydroxybutyl, etc., ketoalkyls, such as 2-ketopropyl, 6-ketoctyl, etc., alkoxy and lower alkenoxy alkyls, such as ethoxyethyl, ethoxypropyl, propoxyethyl, propoxypropyl, diethyleneoxyethyl, triethyleneoxyethyl, tetraethyleneoxyethyl, diethyleneoxyhexyl, etc. The aforementioned acyl groups (C) are such as propionyl, acetyl, etc. The more preferred substituents are hydrogen,  $C_1-C_6$  alkyls and  $C_1-C_6$  hydroxyalkyls.

In a substituted polyamine, the substituents are found at any atom capable of receiving them. The substituted atoms, e.g., substituted nitrogen atoms, are generally geometrically unequivalent, and consequently the substituted amines finding use in the present invention can be mixtures of mono- and poly-substituted polyamines with substituent groups situated at equivalent and/or unequivalent atoms.

The more preferred polyamine finding use within the scope of the present invention is a polyalkylene polyamine,

including alkylene diamine, and including substituted polyamines, e.g., alkyl and hydroxyalkyl-substituted polyalkylene polyamine. Preferably, the alkylene group contains from 2 to 6 carbon atoms, there being preferably from 2 to 3 carbon atoms between the nitrogen atoms. Such groups are exemplified by ethylene, 1,2-propylene, 2,2-dimethylpropylene, trimethylene, 1,3,2-hydroxypropylene, etc. Examples of such polyamines include ethylene diamine, diethylene triamine, di(trimethylene) triamine, dipropylene triamine, triethylene tetraamine, tripropylene tetraamine, tetraethylene pentamine, and pentaethylene hexamine. Such amines encompass isomers such as branched-chain polyamines and previously-mentioned substituted polyamines, including hydroxy- and hydrocarbyl-substituted polyamines. Among the polyalkylene polyamines, those containing 2-12 amino nitrogen atoms and 2-24 carbon atoms are especially preferred, and the C<sub>2</sub>-C<sub>3</sub> alkylene polyamines are most preferred, that is, ethylene diamine, polyethylene polyamine, propylene diamine and polypropylene polyamine, and in particular, the lower polyalkylene polyamines, e.g., ethylene diamine, dipropylene triamine, etc. A particularly preferred polyalkylene polyamine is diethylene triamine.

The amine component of the presently employed fuel additive also may be derived from heterocyclic polyamines, heterocyclic substituted amines and substituted heterocyclic compounds, wherein the heterocycle comprises one or more 5-6 membered rings containing oxygen and/or nitrogen. Such heterocyclic rings may be saturated or unsaturated and substituted with groups selected from the aforementioned (A), (B), (C) and (D). The heterocyclic compounds are exemplified by piperazines, such as 2-methylpiperazine, N-(2-hydroxyethyl)piperazine, 1,2-bis-(N-piperazinyl)ethane and N,N'-bis(N-piperazinyl)piperazine, 2-methylimidazoline, 3-aminopiperidine, 3-aminopyridine, N-(3-aminopropyl)morpholine, etc. Among the heterocyclic compounds the piperazines are preferred.

Typical polyamines that can be used to form the additives employed in this invention by reaction with a polyolefin epoxide include the following: ethylene diamine, 1,2-propylene diamine, 1,3-propylene diamine, diethylene triamine, triethylene tetraamine, hexamethylene diamine, tetraethylene pentamine, dimethylaminopropylene diamine, N-(beta-aminoethyl)piperazine, N-(beta-aminoethyl)piperazine, 3-amino-N-ethylpiperidine, N-(beta-aminoethyl)morpholine, N,N'-di(beta-aminoethyl)piperazine, N,N'-di(beta-aminoethyl)imidazolidone-2, N-(beta-cyanoethyl)ethane-1,2-diamine, 1-amino-3,6,9-triazaoctadecane, 1-amino-3,6-diaza-9-oxadecane, N-(beta-aminoethyl)diethanolamine, N'acetyl methyl-N-(beta-aminoethyl)ethane-1,2-diamine, N-acetyl-1,2-propanediamine, N-(beta-nitroethyl)-1,3-propane diamine, 1,3-dimethyl-5(beta-aminoethyl)hexahydrotriazine, N-(beta-aminoethyl)hexahydrotriazine, 5-(beta-aminoethyl)-1,3,5-dioxazine, 2-(2-aminoethylamino)ethylamino)ethanol, and 2-[2-(2-aminoethylamino)ethylamino]ethanol.

Alternatively, the amine component of the presently employed hydroxyalkyl-substituted amine may be derived from an amine having the formula:



wherein R<sub>1</sub> and R<sub>2</sub> are independently selected from the group consisting of hydrogen and hydrocarbyl of 1 to about 20 carbon atoms and, when taken together, R<sub>1</sub> and R<sub>2</sub> may form one or more 5- or 6-membered rings containing up to about 20 carbon atoms. Preferably, R<sub>1</sub> is hydrogen and R<sub>2</sub> is

a hydrocarbyl group having 1 to about 10 carbon atoms. More preferably, R<sub>1</sub> and R<sub>2</sub> are hydrogen. The hydrocarbyl groups may be straight-chain or branched and may be aliphatic, alicyclic, aromatic or combinations thereof. The hydrocarbyl groups may also contain one or more oxygen atoms.

An amine of the above formula is defined as a "secondary amine" when both R<sub>1</sub> and R<sub>2</sub> are hydrocarbyl. When R<sub>1</sub> is hydrogen and R<sub>2</sub> is hydrocarbyl, the amine is defined as a "primary amine"; and when both R<sub>1</sub> and R<sub>2</sub> are hydrogen, the amine is ammonia.

Primary amines useful in preparing the fuel additives of the present invention contain 1 nitrogen atom and 1 to about 20 carbon atoms, preferably 1 to 10 carbon atoms. The primary amine may also contain one or more oxygen atoms.

Preferably, the hydrocarbyl group of the primary amine is methyl, ethyl, propyl, butyl, pentyl, hexyl, octyl, 2-hydroxyethyl or 2-methoxyethyl. More preferably, the hydrocarbyl group is methyl, ethyl or propyl.

Typical primary amines are exemplified by N-methylamine, N-ethylamine, N-n-propylamine, N-isopropylamine, N-n-butylamine, N-isobutylamine, N-sec-butylamine, N-tert-butylamine, N-n-pentylamine, N-cyclopentylamine, N-n-hexylamine, N-cyclohexylamine, N-octylamine, N-decylamine, N-dodecylamine, N-octadecylamine, N-benzylamine, N-(2-phenylethyl)amine, 2-aminoethanol, 3-amino-1-propanol, 2-(2-aminoethoxy)ethanol, N-(2-methoxyethyl)amine, N-(2-ethoxyethyl)amine and the like. Preferred primary amines are N-methylamine, N-ethylamine and N-n-propylamine.

The amine component of the presently employed fuel additive may also be derived from a secondary amine. The hydrocarbyl groups of the secondary amine may be the same or different and will generally contain 1 to about 20 carbon atoms, preferably 1 to about 10 carbon atoms. One or both of the hydrocarbyl groups may also contain one or more oxygen atoms.

Preferably, the hydrocarbyl groups of the secondary amine are independently selected from the group consisting of methyl, ethyl, propyl, butyl, pentyl, hexyl, 2-hydroxyethyl and 2-methoxyethyl. More preferably, the hydrocarbyl groups are methyl, ethyl or propyl.

Typical secondary amines which may be used in this invention include N,N-dimethylamine, N,N-diethylamine, N,N-di-n-propylamine, N,N-diisopropylamine, N,N-di-n-butylamine, N,N-di-sec-butylamine, N,N-di-n-pentylamine, N,N-di-n-hexylamine, N,N-dicyclohexylamine, N,N-dioctylamine, N-ethyl-N-methylamine, N-methyl-N-n-propylamine, N-n-butyl-N-methylamine, N-methyl-N-octylamine, N-ethyl-N-isopropylamine, N-ethyl-N-octylamine, N,N-di(2-hydroxyethyl)amine, N,N-di(3-hydroxypropyl)amine, N,N-di(ethoxyethyl)amine, N,N-di(propoxyethyl)amine and the like. Preferred secondary amines are N,N-dimethylamine, N,N-diethylamine and N,N-di-n-propylamine.

Cyclic secondary amines may also be employed to form the additives of this invention. In such cyclic compounds, R<sub>1</sub> and R<sub>2</sub> of the formula hereinabove, when taken together, form one or more 5- or 6-membered rings containing up to about 20 carbon atoms. The ring containing the amine nitrogen atom is generally saturated, but may be fused to one or more saturated or unsaturated rings. The rings may be substituted with hydrocarbyl groups of 1 to about 10 carbon atoms and may contain one or more oxygen atoms.

Suitable cyclic secondary amines include piperidine, 4-methylpiperidine, pyrrolidine, morpholine, 2,6-dimethylmorpholine and the like.

In many instances the amine component is not a single compound but a mixture in which one or several compounds predominate with the average composition indicated. For example, tetraethylene pentamine prepared by the polymerization of aziridine or the reaction of dichloroethylene and ammonia will have both lower and higher amine members, e.g., triethylene tetraamine, substituted piperazines and pentaethylene hexamine, but the composition will be mainly tetraethylene pentamine and the empirical formula of the total amine composition will closely approximate that of tetraethylene pentamine. Finally, in preparing the compounds of this invention using a polyamine, where the various nitrogen atoms of the polyamine are not geometrically equivalent, several substitutional isomers are possible and are encompassed within the final product. Methods of preparation of amines and their reactions are detailed in Sidgewick's "The Organic Chemistry of Nitrogen", Clarendon Press, Oxford, 1966; Noller's "Chemistry of Organic Compounds", Saunders, Philadelphia, 2nd Ed., 1957; and Kirk-Othmer's "Encyclopedia of Chemical Technology", 2nd Ed., especially Volume 2, pp. 99-116.

#### Preparation of the Hydroxylalkyl-Substituted Amine Reaction Product

As noted above, the fuel additive finding use in the present invention is a hydroxylalkyl-substituted amine which is the reaction product of (a) a polyolefin epoxide derived from a branched chain polyolefin having an average molecular weight of about 250 to 3,000 and (b) a nitrogen-containing compound selected from ammonia, a monoamine having from 1 to 40 carbon atoms, and a polyamine having from 2 to about 12 amine nitrogen atoms and from 2 to about 40 carbon atoms.

The reaction of the polyolefin epoxide and the amine component is generally carried out either neat or with a solvent at a temperature in the range of about 100° C. to 250° C. and preferably from about 180° C. to about 220° C. A reaction pressure will generally be maintained in the range from about 1 to 250 atmospheres. The reaction pressure will vary depending on the reaction temperature, presence or absence of solvent and the boiling point of the amine component. The reaction usually is conducted in the absence of oxygen, and may be carried out in the presence or absence of a catalyst. The desired product may be obtained by water wash and stripping, usually by aid of vacuum, of any residual solvent.

The mole ratio of basic amine nitrogen to polyolefin epoxide will generally be in the range of about 3 to 50 moles of basic amine nitrogen per mole of epoxide, and more usually about 5 to 20 moles of basic amine nitrogen per mole of epoxide. The mole ratio will depend upon the particular amine and the desired ratio of epoxide to amine. Since suppression of polysubstitution of the amine is usually desired, large mole excesses of the amine will generally be used.

The reaction of polyolefin epoxide and amine may be conducted either in the presence or absence of a catalyst. When employed, suitable catalysts include Lewis acids, such as aluminum trichloride, boron trifluoride, titanium tetrachloride, ferric chloride, and the like. Other useful catalysts include solid catalysts containing both Brønsted and Lewis acid sites, such as alumina, silica, silica-alumina, and the like.

The reaction may also be carried out with or without the presence of a reaction solvent. A reaction solvent is generally employed whenever necessary to reduce the viscosity of

10  
15  
20  
25  
30  
35  
40  
45  
50  
55

the reaction product. These solvents should be stable and inert to the reactants and reaction product. Preferred solvents include aliphatic or aromatic hydrocarbons or aliphatic alcohols.

5 Depending on the temperature of the reaction, the particular polyolefin epoxide used, the mole ratios and the particular amine, as well as the presence or absence of a catalyst, the reaction time may vary from less than 1 hour to about 72 hours.

10 After the reaction has been carried out for a sufficient length of time, the reaction mixture may be subjected to extraction with a hydrocarbon-water or hydrocarbon-alcohol-water medium to free the product from any low-molecular weight amine salts which have formed and any unreacted polyamines. The product may then be isolated by evaporation of the solvent.

15 In most instances, the additive compositions used in this invention are not a pure single product, but rather a mixture of compounds having an average molecular weight. Usually, the range of molecular weights will be relatively narrow and peaked near the indicated molecular weight. Similarly, for the more complicated amines, such as polyamines, the compositions will be a mixture of amines having as the major product the compound indicated as the average composition and having minor amounts of analogous compounds relatively close in compositions to the dominant compound.

#### C. The Hydrocarbyl-Substituted Succinimide

20 The hydrocarbyl-substituted succinimide which can be employed as the aliphatic amine component of the present fuel additive composition is a straight or branched chain hydrocarbyl-substituted succinimide comprising the reaction product of a straight or branched chain hydrocarbyl-substituted succinic acid or anhydride, wherein the hydrocarbyl group has a number average molecular weight of about 250 to 3,000, and a polyamine having from 2 to about 12 amine nitrogen atoms and 2 to about 40 carbon atoms.

25 Preferably, the hydrocarbyl group will have a number average molecular weight in the range of about 700 to 2,200, and more preferably, in the range of about 900 to 1,500. The hydrocarbyl group may be either straight chain or branched chain. Preferably, the hydrocarbyl group will be a branched chain hydrocarbyl group.

30 When employing a branched chain hydrocarbyl-substituted succinimide, the branched chain hydrocarbyl group is preferably derived from polymers of C<sub>2</sub> to C<sub>6</sub> olefins. Such branched chain hydrocarbyl groups are described more fully above in the discussion of hydrocarbyl-substituted amines and hydroxylalkyl-substituted amines. Preferably, the branched chain hydrocarbyl group will be derived from polypropylene or polyisobutylene. More preferably, the branched chain hydrocarbyl group will be derived from polyisobutylene.

35 The succinimides employed in the present invention are prepared by reacting a straight or branched chain hydrocarbyl-substituted succinic acid or anhydride with a polyamine having from 2 to about 12 amine nitrogen atoms and 2 to about 40 carbon atoms.

40 Hydrocarbyl-substituted succinic anhydrides are well known in the art and are prepared by the thermal reaction of olefins and maleic anhydride as described, for example, in U.S. Pat. Nos. 3,361,673 and 3,676,089. Alternatively, hydrocarbyl-substituted succinic anhydrides can be prepared by reaction of chlorinated olefins with maleic anhydride as described, for example, in U.S. Pat. No. 3,172,892. The olefin employed in these reactions has a number average

60

65

molecular weight in the range of about 250 to about 3,000. Preferably, the number average molecular weight of the olefin is about 700 to about 2,200, more preferably about 900 to 1,500.

The reaction of a polyamine with an alkenyl or alkyl succinic acid or anhydride to produce a polyamino alkenyl or alkyl succinimide is well known in the art and is described, for example, in U.S. Pat. Nos. 3,018,291; 3,024,237; 3,172,892; 3,219,666; 3,223,495; 3,272,746; 3,361,673 and 3,443,918.

#### The Amine Component of the Succinimide

The amine moiety of the hydrocarbyl-substituted succinimide is preferably derived from a polyamine having from 2 to about 12 amine nitrogen atoms and from 2 to about 40 carbon atoms. The polyamine is preferably reacted with a hydrocarbyl-substituted succinic acid or anhydride to produce the hydrocarbyl-substituted succinimide fuel additive finding use within the scope of the present invention. The polyamine, encompassing diamines, provides the product succinimide with, on the average, at least about one basic nitrogen atom per succinimide molecule, i.e., a nitrogen atom titratable by strong acid. The polyamine preferably has a carbon-to-nitrogen ratio of from about 1:1 to about 10:1. The polyamine may be substituted with substituents selected from hydrogen, hydrocarbyl groups of from 1 to about 10 carbon atoms, acyl groups of from 2 to about 10 carbon atoms, and monoketone, monohydroxy, mononitro, monocyano, alkyl and alkoxy derivatives of hydrocarbyl groups of from 1 to 10 carbon atoms. It is preferred that at least one of the basic nitrogen atoms of the polyamine is a primary or secondary amino nitrogen. The polyamine component employed in the present invention has been described and exemplified more fully in U.S. Pat. No. 4,191,537.

Hydrocarbyl, as used in describing the amine components used in this invention, denotes an organic radical composed of carbon and hydrogen which may be aliphatic, alicyclic, aromatic or combinations thereof, e.g., aralkyl. Preferably, the hydrocarbyl group will be relatively free of aliphatic unsaturation, i.e., ethylenic and acetylenic, particularly acetylenic unsaturation. The more preferred polyamine finding use within the scope of the present invention is a polyalkylene polyamine, including alkylendiamine, and including substituted polyamines, e.g., alkyl and hydroxy-alkyl-substituted polyalkylene polyamine. Preferably, the alkylene group contains from 2 to 6 carbon atoms, there being preferably from 2 to 3 carbon atoms between the nitrogen atoms. Examples of such polyamines include ethylenediamine, diethylene triamine, triethylene tetramine, di(trimethylene) triamine, dipropylene triamine, tetraethylene pentamine, etc. Among the polyalkylene polyamines, polyethylene polyamine and polypropylene polyamine containing 2-12 amine nitrogen atoms and 2-24 carbon atoms are especially preferred and in particular, the lower polyalkylene polyamines, e.g., ethylenediamine, diethylene triamine, propylene diamine, dipropylene triamine, etc., are most preferred. Particularly preferred polyamines are ethylene diamine and diethylene triamine.

#### Fuel Compositions

The fuel additive composition of the present invention will generally be employed in hydrocarbon fuels to prevent and control engine deposits, particularly intake valve deposits. The proper concentration of the additive composition necessary to achieve the desired level of deposit control

varies depending upon the type of fuel employed, the type of engine, and the presence of other fuel additives.

Generally, the present fuel additive composition will be employed in hydrocarbon fuel in a concentration ranging from about 75 to about 5,000 parts per million (ppm) by weight, preferably from 200 to 2,500 ppm.

In terms of individual components, hydrocarbon fuel containing the fuel additive composition of this invention will generally contain about 50 to 2,500 ppm of the poly(oxyalkylene) hydroxyaromatic ether component and about 25 to 1,000 ppm of the aliphatic amine component. The ratio of the poly(oxyalkylene) hydroxyaromatic ether to aliphatic amine will generally range from about 0.5:1 to about 10:1, and will preferably be about 1:1 or greater.

The fuel additive composition of the present invention may be formulated as a concentrate using an inert stable oleophilic (i.e., dissolves in gasoline) organic solvent boiling in the range of about 150° F. to 400° F. (about 65° C. to 205° C.). Preferably, an aliphatic or an aromatic hydrocarbon solvent is used, such as benzene, toluene, xylene or higher-boiling aromatics or aromatic thinners. Aliphatic alcohols containing about 3 to 8 carbon atoms, such as isopropanol, isobutylcarbinol, n-butanol and the like, in combination with hydrocarbon solvents are also suitable for use with the present additives. In the concentrate, the amount of the additive composition will generally range from about 10 to about 70 weight percent, preferably 10 to 50 weight percent, more preferably from 20 to 40 weight percent.

In gasoline fuels, other fuel additives may be employed with the additives of the present invention, including, for example, oxygenates, such as t-butyl methyl ether, anti-knock agents, such as methylcyclopentadienyl manganese tricarbonyl, and other dispersants/detergents, such as hydrocarbyl amines or succinimides. Additionally, antioxidants, metal deactivators and demulsifiers may be present.

In diesel fuels, other well-known additives can be employed, such as pour point depressants, flow improvers, cetane improvers, and the like.

A fuel-soluble, nonvolatile carrier fluid or oil may also be used with the fuel additive composition of this invention. The carrier fluid is a chemically inert hydrocarbon-soluble liquid vehicle which substantially increases the nonvolatile residue (NVR), or solvent-free liquid fraction of the fuel additive composition while not overwhelmingly contributing to octane requirement increase. The carrier fluid may be a natural or synthetic oil, such as mineral oil, refined petroleum oils, synthetic polyalkanes and alkenes, including hydrogenated and unhydrogenated polyalphaolefins, and synthetic poly(oxyalkylene)-derived oils, such as those described, for example, in U.S. Pat. No. 4,191,537 to Lewis.

These carrier fluids are believed to act as a carrier for the fuel additive composition of the present invention and to assist in removing and retarding deposits. The carrier fluid may also exhibit synergistic deposit control properties when used in combination with the fuel additive composition of this invention.

The carrier fluids are typically employed in amounts ranging from about 100 to about 5000 ppm by weight of the hydrocarbon fuel, preferably from 400 to 3000 ppm of the fuel. Preferably, the ratio of carrier fluid to deposit control additive will range from about 0.5:1 to about 10:1, more preferably from 1:1 to 4:1, most preferably about 2:1.

When employed in a fuel concentrate, carrier fluids will generally be present in amounts ranging from about 20 to about 60 weight percent, preferably from 30 to 50 weight percent.

## 21

## EXAMPLES

The following examples are presented to illustrate specific embodiments of the present invention and synthetic preparations thereof; and should not be interpreted as limitations upon the scope of the invention.

## Example 1

Preparation of  
 $\alpha$ -(4-Benzyloxyphenyl)- $\omega$ -hydroxypoly(oxybutylene)

To a flask equipped with a magnetic stirrer, thermometer, addition funnel, reflux condenser and nitrogen inlet was added 6.88 grams of a 35 wt % dispersion of potassium hydride in mineral oil. Forty grams of 4-benzyloxyphenol dissolved in 500 mL of anhydrous toluene was added dropwise and the resulting mixture was stirred at room temperature for ten minutes. The temperature of the reaction mixture, a thick white suspension, was raised to 90° C. and 430.8 mL of 1,2-epoxybutane was added dropwise. The reaction mixture was refluxed until the pot temperature reached 110° C. (approximately 48 hours) at which time the reaction mixture was a light brown clear solution. The reaction was cooled to room temperature, quenched with 50 mL of methanol and diluted with 1 liter of diethyl ether. The resulting mixture was washed with saturated aqueous ammonium chloride, followed by water and saturated aqueous sodium chloride. The organic layer was dried over anhydrous magnesium sulfate, filtered and the solvents removed in vacuo to yield 390 grams of a yellow oil. The oil was chromatographed on silica gel, eluting with hexane: diethyl ether (1:1), to yield 339.3 grams of the desired product as a colorless oil.

## Example 2

Preparation of  
 $\alpha$ -(4-Hydroxyphenyl)- $\omega$ -hydroxypoly(oxybutylene)

A solution of 54.10 grams of the product from Example 1 in 100 mL of ethyl acetate and 100 mL of acetic acid containing 5.86 grams of 10% palladium on charcoal was hydrogenolyzed at 35–40 psi for 16 hours on a Parr low-pressure hydrogenator. Catalyst filtration and removal of solvent in vacuo followed by azeotropic removal of residual acetic acid with toluene under vacuum yielded 48.1 grams of the desired product as a colorless oil. The product had an average of 24 oxybutylene units.  $^1\text{H}$  NMR ( $\text{CDCl}_3$ )  $\delta$  7.2 (broad s, 2H), 6.7 (s, 4H), 3.1–4.0 (m, 72H), 1.2–1.8 (m, 48H), 0.8 (t, 72H).

Similarly, by using the above procedures and the appropriate starting materials and reagents, the following compounds can be prepared:

$\alpha$ -(2-hydroxyphenyl)- $\omega$ -hydroxypoly(oxybutylene);  
 $\alpha$ -(3-hydroxyphenyl)- $\omega$ -hydroxypoly(oxybutylene);

## 22

- $\alpha$ -(3-t-butyl-4-hydroxyphenyl)- $\omega$ -hydroxypoly(oxybutylene);  
 $\alpha$ -(4-hydroxy-3-methoxyphenyl)- $\omega$ -hydroxypoly(oxybutylene);  
5  $\alpha$ -(3,4-dihydroxyphenyl)- $\omega$ -hydroxypoly(oxybutylene);  
 $\alpha$ -(3,4-hydroxy-5-methylphenyl)- $\omega$ -hydroxypoly(oxybutylene);  
 $\alpha$ -(3,5-di-t-butyl-4-hydroxyphenyl)- $\omega$ -hydroxypoly(oxybutylene); and  
10  $\alpha$ -(3,4,5-trihydroxyphenyl)- $\omega$ -hydroxypoly(oxybutylene).

## Example 3

Preparation of  
 $\alpha$ -(4-Benzyloxyphenyl)- $\omega$ -hydroxypoly(oxypropylene)

To a flask equipped with magnetic stirrer, thermometer, addition funnel, reflux condenser and nitrogen inlet was added 6.88 grams of a 35 wt % dispersion of potassium hydride in mineral oil. 4-Benzyloxyphenol (40 grams) dissolved in 500 mL of anhydrous toluene was added dropwise and then stirred at room temperature for ten minutes. The temperature of the reaction mixture, a thick white suspension, was raised to 110° C. and stirred for 3 hours. The reaction was cooled to room temperature and 349.9 mL of 1,2-epoxypropane was added dropwise. The reaction mixture was refluxed until the pot temperature reached 110° C. (approximately 96 hours) at which time the reaction mixture was a light brown clear solution. The reaction was cooled to room temperature, quenched with 50 mL of methanol and diluted with 1 liter of diethyl ether. The reaction was washed with saturated aqueous ammonium chloride, followed by water and saturated aqueous sodium chloride. The organic layer was dried over anhydrous sulfate, filtered and the solvents removed under vacuum to yield 212.2 grams of the desired product as a light yellow oil.

## Example 4

Preparation of  
 $\alpha$ -(4-Hydroxyphenyl)- $\omega$ -hydroxypoly(oxypropylene)

A solution of 60.0 grams of the product from Example 3 in 100 mL of ethyl acetate and 100 mL of acetic acid containing 7.0 grams of 10% palladium on charcoal was hydrogenolyzed at 35–40 psi for 16 hours on a Parr low-pressure hydrogenator. Catalyst filtration and removal of solvent in vacuo followed by azeotropic removal of the residual acetic acid with toluene under vacuum yielded 31.7 grams of the desired product as a brown oil. The product had an average of 20 oxypropylene units.  $^1\text{H}$  NMR ( $\text{CDCl}_3$ )  $\delta$  6.7 (s, 4H), 5.4–6.0 (broad s, 2H), 3.0–4.0 (m, 60H), 0.8–1.4 (m, 60H).

65 Similarly, by using the above procedures and the appropriate starting materials and reagents, the following compounds can be prepared:

## 23

$\alpha$ -(2-hydroxyphenyl)- $\omega$ -hydroxypoly(oxypropylene);  
 $\alpha$ -(3-hydroxyphenyl)- $\omega$ -hydroxypoly(oxypropylene);  
 $\alpha$ -(4-hydroxy-3-methylphenyl)- $\omega$ -hydroxypoly(oxypropylene);  
 $\alpha$ -(3,5-dimethoxy-4-hydroxyphenyl)- $\omega$ -hydroxypoly(oxypropylene);  
 $\alpha$ -(3,4-dihydroxyphenyl)- $\omega$ -hydroxypoly(oxypropylene);  
 $\alpha$ -(3,5-di-t-butyl-4-hydroxyphenyl)- $\omega$ -hydroxypoly(oxypropylene); and  
 $\alpha$ -(3,4,5-trihydroxyphenyl)- $\omega$ -hydroxypoly(oxypropylene).

## Example 5

## Preparation of 2-(4-Benzylxyloxyphenyl)ethanol

To a flask equipped with a magnetic stirrer, reflux condenser and nitrogen inlet was added 13.8 grams of 2-(4-hydroxyphenyl)ethanol, 14.5 grams of anhydrous potassium carbonate, 33.0 grams of tetrabutylammonium bromide, 12 mL of benzyl chloride and 200 mL of acetone. The reaction mixture was heated at reflux for 3 days, and then cooled to room temperature and filtered. The filtrate was concentrated in vacuo, diluted with 500 mL of dichloromethane, and washed with 2% aqueous sodium hydroxide and then with saturated brine. The organic layer was dried over anhydrous magnesium sulfate, filtered, and concentrated in vacuo. The resulting product was purified by chromatography on silica gel, eluting with dichloromethane, to yield 20.0 grams of the desired product as a white solid.

## Example 6

Preparation of  $\alpha$ -[2-(4-Benzylxyloxyphenyl)ethyl]- $\omega$ -hydroxypoly(oxybutylene)

To a flask equipped with a magnetic stirrer, thermometer, addition funnel, reflux condenser and nitrogen inlet was added 1.05 grams of a 35 weight percent dispersion of potassium hydride in mineral oil and 50 mL of toluene. 2-(4-Benzylxyloxyphenyl)ethanol (6.8 grams) from Example 5, dissolved in 7.5 mL of toluene, was added dropwise and the mixture was heated at reflux for two hours. The reaction was cooled to room temperature and 65 mL of 1,2-epoxybutane were added dropwise. The reaction mixture was then refluxed until the pot temperature reached 110° C. (approximately 16 hours). The reaction was then cooled to room temperature, quenched with 50 mL of methanol and diluted with diethyl ether (300 mL). The organic layer was washed with water (2 times), saturated aqueous ammonium chloride (2 times), dried over anhydrous magnesium sulfate, filtered and concentrated in vacuo. The resulting product was chromatographed on silica gel, eluting with hexane/diethyl ether, followed by hexane/diethyl ether/ethanol (7.5:2.5:0.5) to yield 26.0 grams of the desired product as a colorless oil.

## 24

## Example 7

Preparation of  $\alpha$ -[2-(4-Hydroxyphenyl)ethyl]- $\omega$ -hydroxypoly(oxybutylene)5  
10  
15  
20  
25  
30  
35  
40  
45

A solution of 26.0 grams of the product from Example 6 in 50 mL of ethyl acetate and 50 mL of acetic acid containing 3.0 grams of 10% palladium on charcoal was hydrogenated at 35-40 psi for 16 hours on a Parr low-pressure hydrogenator. Catalyst filtration and removal of solvent in vacuo followed by azeotropic removal of residual acetic acid with toluene under vacuum yielded 21.0 grams of the desired product as a light yellow oil. The product had an average of 38 oxybutylene units.  $^1$ H NMR ( $\text{CDCl}_3$ )  $\delta$  6.7, 6.9 (AB quartet, 4H), 3.0-3.8 (m, 116H), 2.75 (t, 2H), 0.6-1.8 (m, 190H).

Similarly, by using the above procedures and the appropriate starting materials and reagents, the following compounds can be prepared:

$\alpha$ -[2-(2-hydroxyphenyl)ethyl]- $\omega$ -hydroxypoly(oxybutylene);  
 $\alpha$ -[2-(3-hydroxyphenyl)ethyl]- $\omega$ -hydroxypoly(oxybutylene);  
 $\alpha$ -[3-(4-hydroxyphenyl)propyl]- $\omega$ -hydroxypoly(oxybutylene);  
 $\alpha$ -[2-(3,4-dihydroxyphenyl)ethyl]- $\omega$ -hydroxypoly(oxybutylene);  
 $\alpha$ -[3-(3,4-dihydroxyphenyl)propyl]- $\omega$ -hydroxypoly(oxybutylene);  
 $\alpha$ -[2-(3,5-di-t-butyl-4-hydroxyphenyl)ethyl]- $\omega$ -hydroxypoly(oxybutylene); and  
 $\alpha$ -[2-(3,4,5-trihydroxyphenyl)ethyl]- $\omega$ -hydroxypoly(oxybutylene).

## Example 8

Preparation of  $\alpha$ -(4-Hydroxyphenyl)- $\omega$ -benzyloxypoly(oxybutylene)50  
55  
60  
65

To a flask equipped with a magnetic stirrer, thermometer, reflux condenser and nitrogen inlet was added 0.8 grams of a 35 wt % dispersion of potassium hydride in mineral oil. The oil was removed by trituration with anhydrous toluene. The product from Example 2 (6.0 grams) was dissolved in 50 mL of anhydrous tetrahydrofuran and added dropwise to the potassium hydride. The reaction mixture was heated to reflux for 45 minutes and then cooled to room temperature. Benzyl chloride (0.36 mL) was added dropwise and the reaction was then heated to reflux for 12 hours, cooled to room temperature and quenched with 2 mL of isopropanol. The solvent was removed in vacuo and the residue dissolved in 200 mL of diethyl ether, washed with 5% aqueous hydrochloric acid followed by saturated aqueous sodium chloride. The organic layer was dried over anhydrous magnesium sulfate, filtered and the solvents removed under vacuum. The oil was chromatographed on silica gel, eluting

## 25

with hexane/ethyl acetate (7:3), to yield 3.8 grams of the desired product as a colorless oil. The product had an average of 24 oxybutylene units.  $^1\text{H}$  NMR ( $\text{CDCl}_3$ )  $\delta$  7.2–7.4 (m, 6H), 6.7 (s, 4H), 4.4–4.7 (m, 2H), 3.1–4.0 (m, 72H), 1.2–1.8 (m, 48H), 0.8 (t, 72H).

Similarly, by using the above procedures and the appropriate starting materials and reagents, the following compounds can be prepared:

$\alpha$ -(2-hydroxyphenyl)- $\omega$ -benzyloxypoly(oxybutylene);  $\alpha$ -(3-hydroxyphenyl)- $\omega$ -benzyloxypoly(oxybutylene);  $\alpha$ -(3,4-dihydroxyphenyl)- $\omega$ -benzyloxypoly(oxybutylene);  $\alpha$ -(3,5-di-t-butyl-4-hydroxyphenyl)- $\omega$ -benzyloxypoly(oxybutylene);  $\alpha$ -(4-hydroxy-3-methoxyphenyl)- $\omega$ -benzyloxypoly(oxybutylene); and  $\alpha$ -[2-(4-hydroxyphenyl)ethyl]- $\omega$ -benzyloxypoly(oxybutylene).

## Example 9

Preparation of  $\alpha$ -(4-Benzoxypyhenyl)- $\omega$ -docosanoxypropoly(oxybutylene)

To a flask equipped with a magnetic stirrer, addition funnel, reflux condenser and nitrogen inlet was added 7.26 grams of a 35 wt % dispersion of potassium hydride in mineral oil. The oil was removed by trituration with anhydrous hexane, and 500 milliliters of anhydrous tetrahydrofuran were added.  $\alpha$ -(4-Benzoxypyhenyl)- $\omega$ -hydroxypoly(oxybutylene) (104.0 grams) containing an average of 21 oxybutylene units (prepared essentially as described in Example 1), dissolved in 100 milliliters of anhydrous tetrahydrofuran, was added dropwise and the resulting mixture was heated to reflux for two hours. The reaction was then cooled to room temperature and 24.0 grams of 1-bromodocosane were added. The reaction was refluxed for sixteen hours, cooled to room temperature, diluted with 1200 mL of diethyl ether, and washed with 5% aqueous hydrochloric acid, followed by brine. The organic layers were dried over anhydrous magnesium sulfate, filtered and concentrated in vacuo to give an oil. The oil was chromatographed on silica gel, eluting with hexane/ethyl acetate (7:3) to yield 11.0 grams of the desired product as a yellow oil.

## Example 10

Preparation of  $\alpha$ -(4-Hydroxyphenyl)- $\omega$ -docosanoxypropoly(oxybutylene)

A solution of 11.0 grams of the product from Example 9 in 50 mL of ethyl acetate and 50 mL of acetic acid containing 1.5 grams of 10% palladium on charcoal was hydrogenated at 35–40 psi for 14 hours on a Parr low-pressure hydrogenator. Catalyst filtration and removal of solvent in vacuo followed by azeotropic removal of the residual acetic acid with toluene under vacuum yielded 10.2 grams of the

## 26

desired product. The product had an average of 21 oxybutylene units.  $^1\text{H}$  NMR ( $\text{CDCl}_3$ )  $\delta$  6.7 (s, 4H), 3.1–4.0 (m, 62H), 0.6–1.8 (m, 148H).

Similarly, by using the above procedures and the appropriate starting materials and reagents, the following compounds can be prepared:

$\alpha$ -(4-hydroxyphenyl)- $\omega$ -n-butoxypoly(oxybutylene);  $\alpha$ -(4-hydroxyphenyl)- $\omega$ -n-octyloxypoly(oxybutylene);  $\alpha$ -(4-hydroxyphenyl)- $\omega$ -n-dodecyloxypoly(oxybutylene);  $\alpha$ -(3,5-di-t-butyl-4-hydroxyphenyl)- $\omega$ -n-pentyloxypoly(oxybutylene);  $\alpha$ -(4-hydroxy-3-methoxyphenyl)- $\omega$ -n-hexyloxypoly(oxybutylene);  $\alpha$ -(3,4-hydroxyphenyl)- $\omega$ -nonyloxypoly(oxybutylene); and  $\alpha$ -[2-(4-hydroxyphenyl)ethyl]- $\omega$ -octyloxypoly(oxybutylene).

## Example 11

Preparation of  $\alpha$ -(Methanesulfonyl)- $\omega$ -4-dodecylphenoxypropoly(oxybutylene)

To a flask equipped with a magnetic stirrer, septa and a nitrogen inlet was added 35.0 grams of a hydroxy- $\omega$ -4-dodecylphenoxypropoly(oxybutylene) having an average of 19 oxybutylene units (prepared essentially as described in Example 6 of U.S. Pat. No. 4,160,648), 440 mL of dichloromethane and 3.6 mL of triethylamine. The flask was cooled in an ice bath and 1.8 mL of methanesulfonyl chloride were added dropwise. The ice bath was removed and the reaction was stirred at room temperature for 16 hours. Dichloromethane (800 mL) was added and the organic phase was washed two times with saturated aqueous sodium bicarbonate, and then once with brine. The organic layer was dried over anhydrous magnesium sulfate, filtered and concentrated in vacuo to yield 35.04 grams of the desired product as a yellow oil.

## Example 12

Preparation of  $\alpha$ -(4-Benzoxypyhenyl)- $\omega$ -4-dodecylphenoxypropoly(oxybutylene)

To a flask equipped with a magnetic stirrer, reflux condenser, nitrogen inlet and septa was added 2.59 grams of a 35 wt % dispersion of potassium hydride in mineral oil. The mineral oil was removed by trituration with hexane and the flask was cooled in an ice bath. 4-Benzoxypyhenyl (4.11 grams) dissolved in 150 mL of tetrahydrofuran was added dropwise. The ice bath was removed and the reaction was allowed to stir for 45 minutes at room temperature. The mesylate from Example 11 was dissolved in 275 mL of anhydrous tetrahydrofuran and added to the reaction mixture. The resulting solution was refluxed for 16 hours, cooled to room temperature and 10 mL of methanol were added. The reaction was diluted with 1 liter of diethyl ether, washed with water (1

time), brine (1 time), dried over anhydrous magnesium sulfate, filtered and concentrated in vacuo to 36.04 grams of a yellow oil. The oil was chromatographed on silica gel, eluting with hexane/diethyl ether/ethanol (8:1.8:0.2) to yield 18.88 grams of the desired product as a light yellow oil.

## Example 13

Preparation of  $\alpha$ -(4-Hydroxyphenyl)- $\omega$ -4-dodecylphenoxy poly(oxybutylene)

5

A solution of 18.88 grams of the product from Example 12 in 80 mL of ethyl acetate and 80 mL of acetic acid containing 2.08 grams of 10% palladium on charcoal was hydrogenolyzed at 35–40 psi for 6 hours on a Parr low-pressure hydrogenator. Filtration of the catalyst and removal of solvent in vacuo, followed by azeotropic removal of residual acetic acid with toluene under vacuum yielded 17.63 grams of the desired product as a yellow oil. The product had an average of 19 oxybutylene units.  $^1\text{H}$  NMR ( $\text{CDCl}_3$ )  $\delta$  7.0–7.3 (M, 2H), 6.6–6.9 (m, 6H), 4.0–4.2 (m, 1H), 3.8–4.0 (m, 2H), 3.0–3.8 (m, 54H), 0.5–1.8 (m, 120H).

Similarly, by using the above procedures and the appropriate starting materials and reagents, the following compounds can be prepared:

$\alpha$ -(2-hydroxyphenyl)- $\omega$ -4-dodecylphenoxy poly(oxybutylene);  
 $\alpha$ -(3-hydroxyphenyl)- $\omega$ -4-dodecylphenoxy poly(oxybutylene);  
 $\alpha$ -(3,4-dihydroxyphenyl)- $\omega$ -4-dodecylphenoxy poly(oxybutylene);  
 $\alpha$ -(4-hydroxyphenyl)- $\omega$ -phenoxy poly(oxybutylene);  
 $\alpha$ -(4-hydroxyphenyl)- $\omega$ -4-t-butylphenoxy poly(oxybutylene);  
 $\alpha$ -(4-hydroxyphenyl)- $\omega$ -4-decylphenoxy poly(oxybutylene); and  
 $\alpha$ -(4-hydroxyphenyl)- $\omega$ -4-octadecylphenoxy poly(oxybutylene).

## Example 14

Preparation of  $\alpha$ -(4-Benzoxypyhenyl)- $\omega$ -decanoxyloxy poly(oxybutylene)

50

$\alpha$ -(4-Benzoxypyhenyl)- $\omega$ -hydroxypoly(oxybutylene) (40.75 grams) containing an average of 19 oxybutylene units (prepared essentially as described in Example 1) was combined with 200 mL of toluene, 3.9 mL of triethylamine, 1.5 grams of 4-dimethylamine pyridine and 5.2 mL of n-decanoyl chloride in a flask equipped with a thermometer, magnetic stirrer, reflux condenser and nitrogen inlet. The contents were refluxed for 16 hours, cooled to room temperature and diluted with 400 mL of hexane. The organic layers were washed with water (2 times), saturated aqueous sodium bicarbonate (2 times), saturated aqueous sodium chloride (2 times), dried over anhydrous magnesium sulfate,

filtered and concentrated to yield 40 grams of a yellow oil. The oil was chromatographed on silica gel, eluting with hexane/diethyl ether (1:1) to yield 23.3 grams of the product as a yellow oil.

5

## Example 15

Preparation of  $\alpha$ -(4-Hydroxyphenyl)- $\omega$ -decanoxyloxy poly(oxybutylene)

15

A solution of the ester from Example 14 (23.3 grams) in 50 mL of ethyl acetate and 50 mL of acetic acid containing 2.5 grams of 10% palladium on charcoal was hydrogenolyzed at 35–40 psi for 16 hours on a Parr low-pressure hydrogenator. Filtration of the catalyst and removal of solvent in vacuo followed by azeotropic removal of residual acetic acid with toluene under vacuum yielded 16.0 grams of the desired product as a yellow oil. The product had an average of 19 oxybutylene units. IR (neat)  $1735\text{ cm}^{-1}$ ;  $^1\text{H}$  NMR ( $\text{CDCl}_3$ )  $\delta$  6.7 (s, 4H), 4.8–4.9 (m, 1H), 3.1–4.0 (m, 56H), 2.3 (t, 2H), 0.7–1.8 (m, 112H).

Similarly, by using the above procedures and the appropriate starting materials and reagents, the following compounds can be prepared:

$\alpha$ -(2-hydroxyphenyl)- $\omega$ -decanoxyloxy poly(oxybutylene);  
 $\alpha$ -(3-hydroxyphenyl)- $\omega$ -decanoxyloxy poly(oxybutylene);  
 $\alpha$ -(4-hydroxyphenyl)- $\omega$ -dodecanoxyloxy poly(oxybutylene);  
 $\alpha$ -(4-hydroxyphenyl)- $\omega$ -octanoxyloxy poly(oxybutylene);  
 $\alpha$ -(4-hydroxyphenyl)- $\omega$ -butanoxyloxy poly(oxybutylene);  
 $\alpha$ -(4-hydroxyphenyl)- $\omega$ -benzoyloxy poly(oxybutylene);  
 $\alpha$ -(3,4-dihydroxyphenyl)- $\omega$ -hexanoxyloxy poly(oxybutylene);  
 $\alpha$ -(3,4-hydroxyphenyl)- $\omega$ -2-ethylhexanoxyloxy poly(oxybutylene);  
 $\alpha$ -(3,5-di-t-butyl-4-hydroxyphenyl)- $\omega$ -nonanoxyloxy poly(oxybutylene);  
 $\alpha$ -(3,4,5-trihydroxyphenyl)- $\omega$ -decanoxyloxy poly(oxybutylene); and  
 $\alpha$ -[2-(4-hydroxyphenyl)ethyl]- $\omega$ -decanoxyloxy poly(oxybutylene).

40

45

## Example 16

## Single-Cylinder Engine Test

The test compounds were blended in gasoline and their deposit reducing capacity determined in an ASTM/CFR single-cylinder engine test.

A Waukesha CFR single-cylinder engine was used. Each run was carried out for 15 hours, at the end of which time the intake valve was removed, washed with hexane and weighed. The previously determined weight of the clean valve was subtracted from the weight of the valve at the end of the run. The difference between the two weights is the weight of the deposit. A lesser amount of deposit indicates a superior additive. The operating conditions of the test were as follows: water jacket temperature 200° F.; vacuum of 12 in Hg, air-fuel ratio of 12, ignition spark timing of 40° BTC; engine speed is 1800 rpm; the crankcase oil is a commercial 30W oil.

The amount of carbonaceous deposit in milligrams on the intake valves is reported for each of the test compounds in Table I.

TABLE I

| Single-Cylinder Engine Test Results |                                                |       |         |
|-------------------------------------|------------------------------------------------|-------|---------|
| Sample <sup>1</sup>                 | Intake Valve Deposit Weight<br>(in milligrams) |       |         |
|                                     | Run 1                                          | Run 2 | Average |
| Base Fuel                           | 214.7                                          | 193.7 | 204.2   |
| Example 2                           | 12.7                                           | 26.5  | 19.6    |
| Example 4                           | 59.6                                           | 73.8  | 66.7    |
| Example 7                           | 44.3                                           | 54.0  | 42.9    |
| Example 8                           | 52.8                                           | 75.9  | 64.4    |
| Example 10                          | 53.9                                           | 47.9  | 50.9    |
| Example 13                          | 32.2                                           | 32.3  | 32.3    |
| Example 15                          | 32.5                                           | 31.1  | 31.8    |

<sup>1</sup>At 200 parts per million actives (ppma).

The base fuel employed in the above single-cylinder engine tests was a regular octane unleaded gasoline containing no fuel detergent. The test compounds were admixed with the base fuel to give a concentration of 200 ppma (parts per million actives).

The data in Table I illustrates the significant reduction in intake valve deposits provided by the poly(oxyalkylene) hydroxyaromatic ether component of the present fuel additive composition (Examples 2, 4, 7, 8, 10, 13, 15) compared to the base fuel.

### Example 17

#### Multicylinder Engine Test

The fuel additive composition of the present invention was tested in a laboratory multicylinder engine to evaluate its intake valve and combustion chamber deposit control performance. The test engine was a 4.3 liter, TBI (throttle body injected), V6 engine manufactured by General Motors Corporation. The major engine dimensions are set forth in Table II:

TABLE II

| Engine Dimensions   |           |
|---------------------|-----------|
| Bore                | 10.16 cm  |
| Stroke              | 8.84 cm   |
| Displacement Volume | 4.3 liter |
| Compression Ratio   | 9.3:1     |

The test engine was operated for 40 hours (24 hours a day) on a prescribed load and speed schedule representative of typical driving conditions. The cycle for engine operation during the test is set forth in Table III.

TABLE III

| Engine Driving Cycle |                  |                                       |                             |                          |
|----------------------|------------------|---------------------------------------|-----------------------------|--------------------------|
| Step                 | Mode             | Time in<br>Mode<br>[Sec] <sup>1</sup> | Dynamometer<br>Load<br>[kg] | Engine<br>Speed<br>[RPM] |
| 1                    | Idle             | 60                                    | 0                           | 800                      |
| 2                    | City Cruise      | 150                                   | 10                          | 1,500                    |
| 3                    | Acceleration     | 40                                    | 25                          | 2,800                    |
| 4                    | Heavy HWY Cruise | 210                                   | 15                          | 2,200                    |
| 5                    | Light HWY Cruise | 60                                    | 10                          | 2,200                    |

TABLE III-continued

| Engine Driving Cycle |             |                                       |                             |                          |
|----------------------|-------------|---------------------------------------|-----------------------------|--------------------------|
| Step                 | Mode        | Time in<br>Mode<br>[Sec] <sup>1</sup> | Dynamometer<br>Load<br>[kg] | Engine<br>Speed<br>[RPM] |
| 6                    | Idle        | 60                                    | 0                           | 800                      |
| 7                    | City Cruise | 180                                   | 10                          | 1,500                    |
| 8                    | Idle        | 60                                    | 0                           | 800                      |

<sup>1</sup>All steps, except step number 3, include a 15 second transition ramp. Step 3 includes a 20 second transition ramp.

All of the test runs were made with the same base gasoline, which was representative of commercial unleaded fuel. The results are set forth in Table IV.

TABLE IV

| Multicylinder Engine Test Results                        |                 |                                       |                                                |
|----------------------------------------------------------|-----------------|---------------------------------------|------------------------------------------------|
| Sample                                                   | Conc.<br>(ppma) | Intake Valve<br>Deposits <sup>1</sup> | Combustion<br>Chamber<br>Deposits <sup>1</sup> |
| Base Fuel                                                | —               | 972                                   | 1902                                           |
| Poly(oxyalkylene)                                        | 400             | 283                                   | 2547                                           |
| Hydroxyaromatic<br>Ether <sup>2</sup>                    |                 |                                       |                                                |
| Aliphatic Amine/<br>neutral oil <sup>3</sup>             | 200/800         | 291                                   | 2900                                           |
| Poly(oxyalkylene)                                        | 400/200         | 347                                   | 2579                                           |
| Hydroxyaromatic<br>Ether/Aliphatic<br>Amine <sup>4</sup> |                 |                                       |                                                |

<sup>1</sup>Average of two runs, in milligrams (mg).

<sup>2</sup> $\alpha$ -(4-Hydroxyphenyl)- $\omega$ -hydroxypoly(oxybutylene) prepared as described in Example 2.

<sup>3</sup>Mixture of 200 ppm polyisobutyl (MW = 1300) ethylene diamine and 800 ppm of Chevron 500R neutral oil. The polyisobutyl group was derived from Parapol 1300 polyisobutene.

<sup>4</sup>Mixture of 400 ppm of  $\alpha$ -(4-Hydroxyphenyl)- $\omega$ -hydroxypoly(oxybutylene) and 200 ppm of polyisobutyl (MW = 1300) ethylene diamine.

The base fuel employed in the above multicylinder engine tests contained no fuel detergent. The test compounds were admixed with the base fuel at the indicated concentrations.

The data in Table IV demonstrates that the combination of a poly(oxyalkylene) hydroxyaromatic ether and an aliphatic amine gives significantly better intake valve deposit control than the base fuel. Moreover, the data in Table IV further demonstrates that the combination produces fewer combustion chamber deposits than the aliphatic amine component alone.

What is claimed is:

1. A fuel additive composition comprising:

(a) a poly(oxyalkylene) hydroxyaromatic ether having the formula:



or a fuel-soluble salt thereof; wherein

$\text{R}_1$  and  $\text{R}_2$  are each independently hydrogen, hydroxy, lower alkyl having 1 to 6 carbon atoms, or lower alkoxy having 1 to 6 carbon atoms;

$\text{R}_3$  and  $\text{R}_4$  are each independently hydrogen or lower alkyl having 1 to 6 carbon atoms;

$R_5$  is hydrogen, alkyl having 1 to 30 carbon atoms, phenyl, aralkyl or alkaryl having 7 to 36 carbon atoms, or an acyl group of the formula:



5

wherein  $R_6$  is alkyl having 1 to 30 carbon atoms, phenyl, or aralkyl or alkaryl having 7 to 36 carbon atoms;

$n$  is an integer from 5 to 100; and  $x$  is an integer from 0 to 10; and

(b) an aliphatic substituted amine having at least one basic nitrogen atom and containing an aliphatic hydrocarbyl group which has sufficient molecular weight and carbon chain length to render the aliphatic substituted amine soluble in hydrocarbons boiling in the gasoline or diesel range.

2. The fuel additive composition according to claim 1, wherein  $n$  of said poly(oxyalkylene) hydroxyaromatic ether is an integer ranging from 10 to 50.

3. The fuel additive composition according to claim 2, wherein  $n$  of said poly(oxyalkylene) hydroxyaromatic ether is an integer ranging from 15 to 30.

4. The fuel additive composition according to claim 2, wherein  $R_1$  of said poly(oxyalkylene) hydroxyaromatic ether is hydrogen, hydroxy, or lower alkyl having 1 to 4 carbon atoms; and  $R_2$  is hydrogen.

5. The fuel additive composition according to claim 4, wherein  $R_5$  of said poly(oxyalkylene) hydroxyaromatic ether is hydrogen, alkyl having 2 to 22 carbon atoms, alkylphenyl having an alkyl group containing 4 to 24 carbon atoms, or an acyl group having the formula:  $-\text{C}(\text{O})\text{R}_7$ , wherein  $R_7$  is alkyl having 4 to 12 carbon atoms.

6. The fuel additive composition according to claim 5, wherein  $R_1$  of said poly(oxyalkylene) hydroxyaromatic ether is hydrogen or hydroxy.

7. The fuel additive composition according to claim 6, wherein  $R_5$  of said poly(oxyalkylene) hydroxyaromatic ether is hydrogen, alkyl having 4 to 12 carbon atoms, or alkylphenyl having an alkyl group containing 4 to 12 carbon atoms.

8. The fuel additive composition according to claim 7, wherein one of  $R_3$  and  $R_4$  of said poly(oxyalkylene) hydroxyaromatic ether is lower alkyl having 1 to 3 carbon atoms and the other is hydrogen.

9. The fuel additive composition according to claim 8, wherein one of  $R_3$  and  $R_4$  of said poly(oxyalkylene) hydroxyaromatic ether is methyl or ethyl and the other is hydrogen.

10. The fuel additive composition according to claim 9, wherein  $x$  of said poly(oxyalkylene) hydroxyaromatic ether is 0, 1 or 2.

11. The fuel additive composition according to claim 10, wherein  $R_1$  and  $R_5$  of said poly(oxyalkylene) hydroxyaromatic ether are both hydrogen, and  $x$  is 0.

12. The fuel additive composition according to claim 1, wherein said aliphatic substituted amine contains a hydrocarbyl group having a molecular weight in the range of about 250 to about 3,000.

13. The fuel additive composition according to claim 1, wherein said aliphatic substituted amine is selected from the group consisting of:

(1) A straight or branched chain hydrocarbyl-substituted amine having at least one basic nitrogen atom wherein the hydrocarbyl group has a number average molecular weight of about 250 to 3,000;

(2) A hydroxyalkyl-substituted amine comprising the reaction product of (i) a polyolefin epoxide derived from a branched-chain polyolefin having a number average molecular weight of about 250 to 3,000, and (ii) a nitrogen-containing compound selected from ammonia, a monoamine having from 1 to 40 carbon atoms, and a polyamine having from 2 to about 12 amine nitrogen atoms and from 2 to about 40 carbon atoms; and

(3) A straight or branched chain hydrocarbyl-substituted succinimide comprising the reaction product of a straight or branched chain hydrocarbyl-substituted succinic acid or anhydride, wherein the hydrocarbyl group has a number average molecular weight of about 250 to 3,000, and a polyamine having from 2 to about 12 amine nitrogen atoms and 2 to about 40 carbon atoms.

14. The fuel additive composition according to claim 13, wherein the hydrocarbyl or hydroxyalkyl substituent on the aliphatic substituted amine has a number average molecular weight of about 700 to 2,200.

15. The fuel additive composition according to claim 14, wherein the hydrocarbyl or hydroxyalkyl substituent on the aliphatic substituted amine has a number average molecular weight of about 900 to 1,500.

16. The fuel additive composition according to claim 13, wherein the aliphatic substituted amine is a straight or branched chain hydrocarbyl-substituted amine.

17. The fuel additive composition according to claim 16, wherein the aliphatic substituted amine is a branched chain hydrocarbyl-substituted amine.

18. The fuel additive composition according to claim 17, wherein the aliphatic substituted amine is a polyisobutyl amine.

19. The fuel additive composition according to claim 16, wherein the amine moiety of the aliphatic substituted amine is derived from a polyamine having from 2 to 12 amine nitrogen atoms and from 2 to 40 carbon atoms.

20. The fuel additive composition according to claim 19, wherein the polyamine is a polyalkylene polyamine having 2 to 12 amine nitrogen atoms and 2 to 24 carbon atoms.

21. The fuel additive composition according to claim 20, wherein the polyalkylene polyamine is selected from the group consisting of ethylene diamine, diethylene triamine, triethylene tetramine and tetraethylene pentamine.

22. The fuel additive composition according to claim 21, wherein the polyalkylene polyamine is ethylene diamine or diethylene triamine.

23. The fuel additive composition according to claim 13, wherein the aliphatic substituted amine is a hydroxyalkyl-substituted amine.

24. The fuel additive composition according to claim 23, wherein the hydroxyalkyl-substituted amine is derived from a branched chain polyolefin selected from polypropylene or polyisobutene.

25. The fuel additive composition according to claim 24, wherein the branched chain polyolefin is polyisobutene.

26. The fuel additive composition according to claim 23, wherein the hydroxyalkyl-substituted amine is derived from a polyamine having from 2 to about 12 amine nitrogen atoms and 2 to about 40 carbon atoms.

27. The fuel additive composition according to claim 24, wherein the polyamine is a polyalkylene polyamine wherein the alkylene group contains from 2 to 6 carbon atoms and the polyalkylene polyamine contains from 2 to 12 nitrogen atoms and from 2 to 24 carbon atoms.

28. The fuel additive composition according to claim 27, wherein the polyalkylene polyamine is selected from the

group consisting of ethylene diamine, polyethylene polyamine, propylene diamine and polypropylene polyamine.

29. The fuel additive composition according to claim 13, wherein the aliphatic substituted amine is a straight or branched chain hydrocarbyl-substituted succinimide. 5

30. The fuel additive composition according to claim 29, wherein the aliphatic substituted amine is a branched chain hydrocarbyl-substituted succinimide.

31. The fuel additive composition according to claim 30, 10 wherein the branched chain hydrocarbyl substituent is polyisobutyl.

32. The fuel additive composition according to claim 29, wherein the hydrocarbyl-substituted succinimide is derived from a polyalkylene polyamine having 2 to 12 amine nitrogen atoms and 2 to 24 carbon atoms.

33. The fuel additive composition according to claim 32, wherein the polyalkylene polyamine is selected from the group consisting of ethylene diamine, diethylene triamine, triethylene tetramine and tetraethylene pentamine. 15

34. The fuel additive composition according to claim 33, wherein the polyalkylene polyamine is ethylene diamine or diethylene triamine.

35. A fuel composition comprising a major amount of hydrocarbons boiling in the gasoline or diesel range and an effective detergent amount of a fuel additive composition comprising: 20

(a) a poly(oxyalkylene) hydroxyaromatic ether having the formula:



or a fuel-soluble salt thereof; wherein R<sub>1</sub> and R<sub>2</sub> are each independently hydrogen, hydroxy, lower alkyl having 1 to 6 carbon atoms, or lower alkoxy having 1 to 6 carbon atoms; 40 R<sub>3</sub> and R<sub>4</sub> are each independently hydrogen or lower alkyl having 1 to 6 carbon atoms; R<sub>5</sub> is hydrogen, alkyl having 1 to 30 carbon atoms, phenyl, aralkyl or alkaryl having 7 to 36 carbon atoms, or an acyl group of the formula: 45



wherein R<sub>6</sub> is alkyl having 1 to 30 carbon atoms, phenyl, or aralkyl or alkaryl having 7 to 36 carbon atoms; n is an integer from 5 to 100; and x is an integer from 55 0 to 10; and

(b) an aliphatic substituted amine having at least one basic nitrogen atom and containing an aliphatic hydrocarbyl group which has sufficient molecular weight and carbon chain length to render the aliphatic substituted amine soluble in hydrocarbons boiling in the gasoline or diesel range. 60

36. The fuel composition according to claim 35, wherein R<sub>1</sub> of said poly(oxyalkylene) hydroxyaromatic ether is hydrogen, hydroxy, or lower alkyl having 1 to 4 carbon atoms; R<sub>2</sub> is hydrogen; one of R<sub>3</sub> and R<sub>4</sub> is hydrogen and the other is methyl or ethyl; R<sub>5</sub> is hydrogen, alkyl having 2 to 65

22 carbon atoms, alkylphenyl having an alkyl group containing 4 to 24 carbon atoms, or an acyl group having the formula: —C(O)R<sub>7</sub>, wherein R<sub>7</sub> is alkyl having 4 to 12 carbon atoms; n is 15 to 30; and x is 0, 1 or 2.

37. The fuel composition according to claim 36, wherein R<sub>1</sub> of said poly(oxyalkylene) hydroxyaromatic ether is hydrogen or hydroxy; R<sub>5</sub> is hydrogen, alkyl having 4 to 12 carbon atoms, or alkylphenyl having an alkyl group containing 4 to 12 carbon atoms; and x is 0. 15

38. The fuel composition according to claim 37, wherein R<sub>1</sub> and R<sub>5</sub> of said poly(oxyalkylene) hydroxyaromatic ether are both hydrogen.

39. The fuel composition according to claim 35, wherein said aliphatic substituted amine is a polyisobutyl substituted amine.

40. The fuel composition according to claim 39, wherein the amine moiety is derived from a polyamine having from 2 to 12 amine nitrogen atoms and from 2 to 40 carbon atoms. 20

41. The fuel composition according to claim 40, wherein said polyamine is selected from the group consisting of ethylenediamine, propylenediamine, diethylenetriamine and dipropylenetriamine.

42. The fuel composition according to claim 41, wherein the polyamine is ethylenediamine or diethylenetriamine.

43. The fuel composition according to claim 35, wherein said composition contains about 50 to about 2,500 parts per million by weight of said poly(oxyalkylene) hydroxyaromatic ether and about 25 to about 1,000 parts per million of said aliphatic substituted amine.

44. A fuel concentrate comprising an inert stable oleophilic organic solvent boiling in the range of from about 150° F. to 400° F. and from about 10 to about 70 weight percent of a fuel additive composition comprising:

(a) a poly(oxyalkylene) hydroxyaromatic ether having the formula:



or a fuel-soluble salt thereof; wherein R<sub>1</sub> and R<sub>2</sub> are each independently hydrogen, hydroxy, lower alkyl having 1 to 6 carbon atoms, or lower alkoxy having 1 to 6 carbon atoms; R<sub>3</sub> and R<sub>4</sub> are each independently hydrogen or lower alkyl having 1 to 6 carbon atoms; R<sub>5</sub> is hydrogen, alkyl having 1 to 30 carbon atoms, phenyl, aralkyl or alkaryl having 7 to 36 carbon atoms, or an acyl group of the formula: 50



wherein R<sub>6</sub> is alkyl having 1 to 30 carbon atoms, phenyl, or aralkyl or alkaryl having 7 to 36 carbon atoms; n is an integer from 5 to 100; and x is an integer from 0 to 10; and

(b) an aliphatic substituted amine having at least one basic nitrogen atom and containing an aliphatic hydrocarbyl group which has sufficient molecular weight and carbon chain length to render the aliphatic substituted amine soluble in hydrocarbons boiling in the gasoline or diesel range. 60

45. The fuel concentrate according to claim 44, wherein R<sub>1</sub> of said poly(oxyalkylene) hydroxyaromatic ether is hydrogen, hydroxy, or lower alkyl having 1 to 4 carbon atoms; R<sub>2</sub> is hydrogen; one of R<sub>3</sub> and R<sub>4</sub> is hydrogen and the other is methyl or ethyl; R<sub>5</sub> is hydrogen, alkyl having 2 to 22 carbon atoms, alkylphenyl having an alkyl group containing 4 to 24 carbon atoms, or an acyl group having the formula: —C(O)R<sub>7</sub>, wherein R<sub>7</sub> is alkyl having 4 to 12 carbon atoms; n is 15 to 30; and x is 0, 1 or 2.

46. The fuel concentrate according to claim 45, wherein R<sub>1</sub> of said poly(oxyalkylene) hydroxyaromatic ether is hydrogen or hydroxy; R<sub>5</sub> is hydrogen, alkyl having 4 to 12 carbon atoms, or alkylphenyl having an alkyl group containing 4 to 12 carbon atoms; and x is 0.

47. The fuel concentrate according to claim 46, wherein R<sub>1</sub> and R<sub>5</sub> of said poly(oxyalkylene) hydroxyaromatic ether are both hydrogen.

5

10

15

48. The fuel concentrate according to claim 44, wherein said aliphatic substituted amine is a polyisobutyl substituted amine.

49. The fuel concentrate according to claim 48, wherein the amine moiety is derived from a polyamine having from 2 to 12 amine nitrogen atoms and from 2 to 40 carbon atoms.

50. The fuel concentrate according to claim 49, wherein said polyamine is selected from the group consisting of ethylenediamine, propylenediamine, diethylenetriamine and dipropylenetriamine.

51. The fuel concentrate according to claim 50, wherein the polyamine is ethylenediamine or diethylenetriamine.

\* \* \* \* \*